

# United States Patent [19]

Massey et al.

[11]

4,377,392

[45]

Mar. 22, 1983

[54] COAL COMPOSITION

[75] Inventors: Lester G. Massey, Moreland Hills, Ohio; Robert I. Brabets, Lombard; William A. Abel, Joliet, both of Ill.

[73] Assignee: CNG Research Company, Cleveland, Ohio

[21] Appl. No.: 295,755

[22] Filed: Aug. 24, 1981

Related U.S. Application Data

[63] Continuation-in-part of Ser. No. 261,470, May 7, 1981, Pat No. 4,364,740, which is a continuation-in-part of PCT/US81/00273, Mar. 4, 1981, WO81/02583, abandoned, which is a continuation-in-part of Ser. No. 127,740, Mar. 6, 1980, Pat. No. 4,313,737.

[51] Int. Cl.<sup>3</sup> ..... C10L 1/32; C10L 9/08

[52] U.S. Cl. ..... 44/51; 44/1 C

[58] Field of Search ..... 44/1 C, 1 SR, 51; 241/2, 17, 23, 24, 16; 209/160

[56] References Cited

U.S. PATENT DOCUMENTS

|           |        |                  |         |
|-----------|--------|------------------|---------|
| 2,560,807 | 7/1951 | Lobo             | 241/1   |
| 2,568,400 | 9/1951 | Kearby           | 241/5   |
| 3,660,054 | 5/1972 | Rieve            | 44/1 SR |
| 3,756,791 | 9/1973 | Mancke           | 44/1 SR |
| 3,897,010 | 7/1975 | Weishaupt et al. | 241/5   |
| 3,973,733 | 8/1976 | Switzer          | 241/1   |
| 4,030,893 | 6/1977 | Keller           | 44/1 SR |
| 4,192,651 | 3/1980 | Keller           | 44/1 SR |

OTHER PUBLICATIONS

R. A. Glenn et al., "A Study of Ultrafine Coal Pulveri-

zation and its Application", pp. 20, 90, (Oct. 1963), U.S. Dept. of Commerce, Springfield, VA.

Shao Lee Soo et al., "Final Report and Evaluation of the ILOK-4-Micron Coal Grinding Process," Univ. of Illinois, Urbana-Champaign, Ill., (Dec. 1976).

Primary Examiner—Carl F. Dees  
Attorney, Agent, or Firm—Allegretti, Newitt, Witcoff & McAndrews

[57]

ABSTRACT

A shattered hydrocarbonaceous product comprising a mixture of discrete comminuted hydrocarbonaceous particles having a volumetric mean particle size equivalent to less than about 5 microns in diameter separate from or in admixture with discrete inorganic and mineral particles having a mean particle size substantially the same as in the unshattered original solid is disclosed. The shattered product is produced by the explosive comminution of a slurry of fluid permeable hydrocarbonaceous solid which was heated and pressurized to supercritical conditions and then permitted to suddenly expand. The product hydrocarbonaceous fraction is substantially scissioned from the mineral fraction and has a lower density, greater solvent solubility and different reactivity to oxygen than does the feed solid. This hydrocarbonaceous fraction also includes a subfraction of particles having a particle size, by volume distribution, of less than about 2 microns in diameter which contain substantially no sulfur compounds. In addition, the product hydrocarbonaceous fraction has a solubility in methanol at least about twice that of a product produced by explosive comminution at subcritical conditions.

10 Claims, 13 Drawing Figures



Fig. 4



Fig. 2



Fig. 3







Fig. 6

## *HEATER SYSTEM*



Fig. 7

Fig. 8

AIR OXIDATION THERMOGRAMS



Fig. 11



Fig. 12



FIG. 13



## COAL COMPOSITION

## CROSS REFERENCE TO RELATED APPLICATIONS

This application is a continuation-in-part of Ser. No. 261,470, May 7, 1981, Pat. No. 4,364,740, which is a continuation-in-part of PCT/US 81/00273, Mar. 4, 1981, published as WO81/02583 on Sep. 17, 1981, abandoned, which is a continuation-in-part of Ser. No. 127,740, Mar. 6, 1980, Pat. No. 4,313,737.

## BACKGROUND OF THE INVENTION

The expanding need for energy combined with the depletion of known crude oil reserves has created a serious need for the development of alternatives to crude oil as an energy source. One of the most abundant energy sources, particularly in the United States, is coal. Estimates have been made which indicate that the United States has enough coal to satisfy its energy needs for the next two hundred years. Much of the available coal, however, contains significant amounts of inorganic ash forming minerals, such as quartz and clay, and sulfur compounds, such as pyrites and organic compounds in admixture with the hydrocarbonaceous portion of the coal, which create serious pollution problems when burned. The amount of sulfur and ash forming mineral components in coal varies. However, virtually all types of coal contain such impurities and potential pollutants to some degree entrapped within the coal as mined. As a result, expensive pollution control equipment is usually required as part of any installation using coal as a fuel. The added cost of this equipment seriously detracts from and restricts the use of coal as an energy source.

To overcome the pollution problems associated with the combustion of coal, techniques have been developed for converting coal into liquids or gases from which the potential pollutants, e.g., sulfur, can be removed. For example, coal can be gasified into methane, water gas, and other combustible gases whereby the mineral matter contained in the coal is substantially removed during the gasification process. The sulfur containing pollutants, however, still remain in the resultant gaseous products and must be removed from these products by a separate processing step.

U.S. Pat. No. 3,850,738 issued to Stewart, Jr. et al provides another example of the conversion of coal to more valuable products. In this process, coal is contacted with water at high temperatures and pressures to 50 thermally crack the hydrocarbonaceous material in the coal into aralkanes, gaseous hydrocarbons and undissolved ash.

Another technique for increasing the availability and use of raw coal involves the comminution of coal into a fine particle size in an effort to separate the coal into discrete component parts. One method of comminution, known as chemical comminution is illustrated in U.S. Pat. No. 3,850,477 issued to Aldrich et al involves weakening the intermolecular forces of the coal particles by anhydrous ammonia or other suitable chemicals.

Another method of comminution involves mechanical comminution or grinding. In this method, the grinding is effected by ball or jet milling or any other techniques wherein the coal particles impinge against or are contacted with a solid obstruction. Jet milling, for example, involves entraining coal particles in a gas stream at high velocity and directing the gas stream against a

solid obstruction. Examples of jet milling are shown and described in Switzer, U.S. Pat. No. 3,973,733 and Weishaupt et al, U.S. Pat. No. 3,897,010. Specific examples of such jet milling devices include the "Micronizer" brand fluid energy mill manufactured by Sturtevant Mill Company and the "Jet-O-Mizer" fluid energy reduction mill produced by the Fluid Energy Processing and Equipment Company. These devices are described in an article, R. A. Glenn et al, A Study of Ultra-fine

15 brand fluid energy mill manufactured by Sturtevant Mill Company and the "Jet-O-Mizer" fluid energy reduction mill produced by the Fluid Energy Processing and Equipment Company. These devices are described in an article, R. A. Glenn et al, A Study of Ultra-fine 10 Coal Pulverization and its Application, pp. 20, 90 (October 1963), distributed by the National Technical Information Service, U.S. Department of Commerce, 5285 Port Royal Road, Springfield, Va. 22151. Mechanical comminution techniques are frequently used, for example, to provide feed coal to a gasification reactor.

Ball milling, jet milling and other mechanical impingement techniques involve relatively crude forms of comminution. First, and most importantly, these techniques do not comminute selectively; that is, they comminute the ash forming minerals as well as the valuable hydrocarbon portion of the coal. Another disadvantage is that the mechanical or grinding techniques do not separate or scission the hydrocarbonaceous matter within the coal from the mineral constituents of the coal. That is, ash forming minerals generally remain physically attached to the hydrocarbonaceous material in the coal, after milling, to a considerable extent. The minerals thus cannot be removed from the desired hydrocarbonaceous particles. In addition, organic forms of sulfur remain chemically bonded in the hydrocarbon. As a result, it is difficult to isolate the hydrocarbon from the pollutants. Second, these techniques are limited in their degree of size reduction. Ball milling and jet milling and other mechanical impingement techniques cannot effectively comminute coal, for example, to a mean particle size of less than about 2 microns<sup>1</sup> because of the inherent elasticity of the coal.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880

which is combined with a jet milling reactor to produce a final product with mean particle diameter of about 5 microns. Explosive comminution is also taught in Snyder, U.S. Pat. No. 3,895,760; and Ribas, U.S. Pat. No. 3,881,660.

Finally, the Jet Propulsion Laboratory (JPL) in Pasadena, Ca. has also conducted research on the feeding of coal into high pressure reactors. This research involves plasticizing solid coal at high temperatures and pressures, then screw extruding the resultant mass at high pressure through a nozzle. Fine particles are, as a result, sprayed into a reactor. This work is described in "Technical Support Package on Screw-Extruded Coal Continuous Coal Processing Method and Means," for NASA Tech. Brief, Winter 1977 (updated April 1978), Vol. 2, No. 4, Item 33, prepared by W. P. Butler.

#### SUMMARY OF THE INVENTION

It is an object of the present invention to provide a novel form of solid hydrocarbonaceous matter from a naturally occurring hydrocarbonaceous solid containing an admixture of hydrocarbonaceous components and mineral components, such as coal, wherein this novel form of hydrocarbonaceous solid has both chemical and physical properties different from the hydrocarbonaceous solid from which it was produced and a reduced mineral concentration.

We have discovered that there is an advantage associated with the explosive comminution of porous hydrocarbonaceous solids such as coal which can be used to produce selective comminution of the hydrocarbonaceous particles from the mineral particles. Specifically, the hydrocarbonaceous component is a porous, fluid-permeable solid whereas the mineral component is a relatively crystalline, fluid-impervious solid. As a result, the hydrocarbonaceous components of the hydrocarbonaceous solids, e.g. coal, are the only components of the solid which are comminuted by an explosive comminution of the solid. It has been discovered that if certain conditions are employed in the explosive comminution of a hydrocarbonaceous solid such as coal, the mineral particles in the coal are scissioned from the hydrocarbonaceous components contained therein and that ultrafine hydrocarbonaceous particles are produced without substantially reducing the size of the mineral matter within the coal. This permits the isolation or fractionation of the valuable hydrocarbonaceous particles from the undesirable ash-forming and pollutant-forming mineral particles.

A preferred embodiment of the present invention comprises the product of the rapid, e.g. explosive, expansion of a slurry of a hydrocarbonaceous solid, e.g. coal, and a fluid or liquid initially maintained at supercritical temperatures and pressures. Supercritical conditions are necessary so that the fluid, e.g. water or a low molecular weight alcohol such as methanol, which fills the coal pores becomes a high energy, dense fluid. The dense fluid mass forms a column of fluid within the pores of the coal, the inertia of which is sufficient to prevent the fluid from gradually escaping the pores during the extremely rapid, e.g. instantaneous, depressurization. As a result, the fluid expands rapidly, if not instantaneously, thereby causing the coal to literally explode. Less dense fluids, e.g. vapors, at subcritical temperatures and pressures do not have sufficient mass and energy to fully provide this effect. For example, although water vapor maintained in the pores of the coal at subcritical conditions will provide some shatter-

ing, the mean particle size of the resulting product remains relatively large and, as a result, there is little scissioning of the hydrocarbonaceous components from the mineral components of the coal in comparison to the results obtained by explosions from supercritical conditions.

As used in the description of a preferred embodiment of the present invention, the "critical point" of a liquid refers to the temperature and pressure at which the vapor phase and the liquid phase of the liquid can no longer be distinguished, i.e. the phases merge. "Critical temperature" refers to the temperature of the liquid-vapor at the critical point, that is, the temperature above which the substance cannot be liquefied at any pressure. "Critical pressure" refers to the vapor pressure of the liquid at the critical temperature. "Critical phenomena" refers to the physical properties of liquid and gases at the critical point. A liquid which has been pressurized above its critical pressure and heated above its critical temperature will be referred to as a "supercritical fluid." The critical point of water occurs at about 3205 psia and about 705° F.

The explosive comminution of coal according to the preferred embodiment of the present invention requires the formation of a mixture of coal and sufficient fluid water or low molecular weight alcohol to permit the fluid to permeate the pores of the coal such as is obtained by the formation of a slurry of coal and water or alcohol.

The pressure and temperature to which the slurry is subjected are preferably less than about 16,000 psia and about 1,000° F., respectively. These upper limits, however, are primarily determined by design safety considerations based on known current materials and methods of construction only. Preferred pressures are between about 4,000 psia and about 16,000 psia. Particularly preferred pressures are between about 6,000 psia and about 15,000 psia. Preferred temperatures are between 750° F. and 950° F.

The slurry is preferably maintained at the preferred temperature and pressure for a short period of time. The exact time is determined primarily by the exact temperature and pressure imposed on the slurry. At the preferred operating conditions, the time period is less than about 15 seconds. In any event, the time should not permit the fluid, e.g. water or low molecular weight alcohol to dissolve the mineral components of the coal to a substantial degree.

Finally, the pressure of the slurry is rapidly reduced from the initial pressure imposed on it to a second predetermined pressure. The second predetermined pressure is substantially below the critical pressure of the fluid, preferably near ambient pressure, i.e. less than about 75 psia. The temperature of the slurry drops, as a result of the energy associated with the expansion of the fluid, to a second predetermined temperature and preferably above the dew point of the fluid, e.g., water or low molecular weight alcohol, at the second pressure. At ambient pressure, the preferred temperature is above about 250° F. and is preferably about 260°-300° F. The reduction in pressure is substantially instantaneous so that the pressurized fluid within the coal pores cannot escape gradually. Preferably, the pressure reduction takes place within less than about 100 microseconds, more preferably within less than about 10 microseconds and most preferably within less than about 1 microsecond to thereby effectively shatter the coal and to pro-

vide a hydrocarbonaceous fraction readily separable from the mineral fraction of the coal.

In a further embodiment, the present invention provides a material produced from the selective supercritical comminution of coal having distinct, separable fractions comprising a hydrocarbonaceous fraction consisting essentially of discrete particles of hydrocarbonaceous material having a volumetric mean particle size of less than about 5 microns in diameter and a mineral fraction consisting essentially of discrete particles of mineral matter having a volumetric mean particle size substantially unchanged from the original material. Typically, the volumetric mean particle size of the minerals is greater than about 5 microns in diameter in both the original material and the comminuted material.

In a specific embodiment of the present invention, a hydrocarbonaceous material derived from coal is provided, being relatively free of mineral components and having a volumetric mean particle size of less than about 5 microns. This material is further characterized as having a density of about 0.7 to about 0.9 grams per cubic centimeter, i.e. about 50 to about 75% of the density of known forms of coal; a solubility in a solvent, selected from the group consisting of gasoline, benzene, methyl alcohol, carbon tetrachloride and tetralin, about 2 times to about 6 times greater than the solubility of the original coal; a subfraction of discrete hydrocarbonaceous particles substantially free of sulfur and having a particle size of less than about 2 microns in diameter; and an oxidation decomposition rate, determined by thermogravimetric analysis at ambient atmosphere, which includes a first peak at about 300° C. and a second peak between about 350° and 450° C. wherein the decomposition rate decreases to substantially zero between the first and second peaks. The reactivity to oxygen is distinctly greater than for the untreated coal.

In addition, the hydrocarbonaceous material is scissioned from the mineral material and has a solubility in methanol of at least about twice that of a product produced at subcritical temperatures and pressures. These and other objects, advantages and features of the invention will be set forth in the detailed description which follows.

#### BRIEF DESCRIPTION OF THE DRAWINGS

In the detailed description which follows, reference will be made to the following figures:

FIG. 1 is a block diagram of the basic steps utilized in a preferred embodiment of the process of the present invention.

FIG. 2 is a graph showing the volumetric mean particle size of the explosively shattered product of Illinois-6 coal as a function of temperature and pressure.

FIG. 3 is a graph of the volumetric mean particle size of explosively shattered Pittsburgh coal as a function of temperature and pressure.

FIG. 4 is a graph showing the product size distribution for an explosively shattered Illinois-6 coal at specific temperatures and pressures in accordance with the present invention.

FIG. 5 is a detailed schematic view of a preferred embodiment of the process of the present invention.

FIG. 6 is a detailed schematic view of a preferred heater design for use in the process of the present invention.

FIG. 7 is a graph comparing the decomposition rates of raw, feed Illinois-6 coal and the explosively shattered

product produced in accordance with the present invention.

FIG. 8 is a graph comparing the decomposition rates of raw, feed Pittsburgh-8 coal and the explosively shattered product produced in accordance with the present invention.

FIG. 9 is a graph comparing high performance liquid chromatographs of methanol extracts of Illinois-6 coal prepared from (a) raw feed, (b) a prior art ball milled product and (c) an explosively shattered product produced in accordance with the present invention.

FIG. 10 is a graph comparing high performance liquid chromatographs of methanol extracts of Pittsburgh-8 coal prepared from (a) raw feed, (b) a prior art ball milled product and (c) an explosively shattered product produced in accordance with the present invention.

FIG. 11 is a plot graphically representing the various data points utilized while conducting experiments comparing the supercritical fluid thermodynamic regime comprising the present invention with the prior art thermodynamic regimes of superpressured water and superheated steam.

FIG. 12 graphically represents and compares the correlations obtained for the superpressured water and supercritical fluid thermodynamic regimes for the data points set forth in FIG. 11.

FIG. 13 graphically represents and compares the correlations obtained for the superheated steam and supercritical fluid thermodynamic regimes for the data points set forth in FIG. 11.

#### DESCRIPTION OF THE PREFERRED EMBODIMENT

##### General Description of the Preferred Process and Apparatus Used Therein

Referring to a preferred embodiment of the process of the present invention, as illustrated in block diagram form in FIG. 1, a slurry of a liquid, such as water or a low molecular weight alcohol such as methanol, ethanol, propanol or isopropanol and a solid hydrocarbonaceous material, such as coal is prepared in a mixing and storage unit 12. The hydrocarbonaceous solid is preferably coal, but could also be oil shale or any other porous or fluid-permeable, friable hydrocarbonaceous solid containing an admixture of hydrocarbonaceous particles and mineral particles. The quantity of liquid added to unit 12 is an amount sufficient to fill the pores and cavities of the coal, preferably by first forming a true slurry, i.e. enough liquid to fill the pores of the solid and the interstitial spaces between the solid particles, producing a mixture having fluid characteristics for ease in handling.

An electrolyte is preferably added to the slurry by control unit 13. The electrolyte is preferably a solution of hydroxide salts having a basic pH, such as sodium hydroxide, calcium hydroxide or ammonium hydroxide. The electrolyte provides a method of controlling the temperature of the reactor and to increase the temperature operating range.

In addition to temperature control, the electrolyte addition also aids in avoiding coal agglomerating at high temperatures. It is known that coals have a strong tendency to agglomerate at temperatures above their softening point. It has recently been reported that the melting point of coal can be raised by contact with calcium hydroxide due to an undefined reaction between the coal and the calcium ion. Feldman et al.,

Summary Report on A Novel Approach to Coal Gasification Using Chemically Incorporated CaO, Nov. 11, 1977 (Battelle Memorial Institute, Columbus, Ohio). In contrast, we believe that the reaction which is involved takes place between the hydroxide ion and the substances known as macerals, which melt and become sticky as the coal is heated above its softening point. In any event, we have discovered that by increasing the pH of the slurry, such as by adding basic hydroxide ion, the slurry can be heated somewhat beyond the normal melting point of the coal without agglomerating of the coal particles.

As indicated in FIG. 1, the slurry is passed, as needed, to a feed system 14 which preferably delivers the feed at a constant pressure equal to the desired operating pressure of the heating zone. By delivering the slurry at a constant pressure, the feed pumping system 14 counteracts or compensates for pressure changes within the process. The rate at which slurry is delivered decreases as the pressure increases and vice versa. Pressurization in combination with the high temperature forces the water into the pores of the normally hydrophobic coal. The desired pressure is greater than the critical pressure of the liquid which is used to make the slurry, i.e. for water about 3200 psia, and less than about 16,000 psia, preferably between about 4,000 and about 16,000 psia. The upper limit of the reactor operating pressure is determined principally by the temperature and pressure rated capacity of the apparatus components.

The pressurized slurry is then delivered to a heating chamber 16 wherein the temperature of the slurry is raised to a predetermined temperature above the critical temperature of the liquid which in the case of water is about 705° F., and preferably below about 1000° F. Particularly preferred temperatures are between about 750° F. and about 950° F. The supercritical temperatures and pressures produce a supercritical fluid which penetrates and thus saturates the coal pores with a high energy compressed fluid.

Although many methods may be used to heat the slurry, heating chamber 16 preferably comprises an electrode positioned within a chamber adapted to operate at high temperatures and pressures. As slurry is passed through the chamber, an electrical current is passed from the electrode through the slurry to the chamber wall. The resistance of the slurry is thus used as a method of directly heating the slurry passed to heating chamber 16.

The temperature at which coal begins to agglomerate varies between about 650° and about 825° F. and is a function of the type of coal being heated. As stated, this agglomeration can be reduced to some degree by the addition of hydroxide ion. In addition, agglomeration in heating chamber 16 can be minimized or avoided, without adding hydroxide, by using a slurry with low solids content, preferably less than about 15 to 25 by weight percent solids.

The pressurized, heated slurry is held in a chamber 18 for a predetermined length of time sufficient to insure penetration and saturation of the supercritical water into the pores and interstices of the coal. The optimum residence time is dependent on the temperature and pressure as well as the size of the coal particles, and the type of coal used in making the slurry. Preferred residence times are less than 15 seconds in the preferred pressure and temperature range. It has been discovered that increasing the residence time up to about 15 seconds increases the degree of comminution up to a cer-

tain point, and that increasing the residence time beyond 15 seconds has no added or improved effect. In fact, long residence times are to be generally avoided because they may lead to undesired solvation of the coal, reduced shattering, and dissolution of the minerals in the coal and/or cause undesired chemical reactions.

The heated and pressurized slurry is then passed to an expansion unit 20 wherein the high pressure imposed on the slurry is reduced rapidly, preferably in a substantially instantaneous fashion. The pressure to which the slurry is reduced is below the critical pressure of the liquid and is preferably about ambient pressure, i.e. about 75 psia or lower. The temperature of the slurry drops as a result of the adiabatic expansion of the fluid in the slurry. Preferably, however, the temperature drop is controlled to provide a temperature above the dew point of the water at the second pressure to prevent vapor condensation which can interfere with subsequent separation steps. Particularly preferred final temperatures after expansion are about 250° F.

The expansion unit preferably includes a high pressure adiabatic expansion orifice having a small opening sufficient to permit the coal particles to pass without plugging. The design of the orifice includes an opening which provides for passage of the slurry across the opening in less than about 10 microseconds, preferably in less than about 1 microsecond. The design of this orifice insures that the reduction in the pressure imposed on the coal will occur substantially instantaneously, preferably in less than 100 microseconds. Particularly preferred times for this pressure reduction are less than about 10 microseconds and most particularly preferred are less than about 1 microsecond.

The time required for the slurry to pass from supercritical pressures to the lower preferably ambient pressure is as short as possible so that the high pressure of fluid in the pores is prevented from being gradually released or "leaking" from the pores. The more rapid the depressurization, the more the coal is comminuted since the potential energy of fluid expansion contained in the pores of the coal is not prematurely lost.

It has also been discovered that if the coal impinges on an obstruction near the orifice opening, the selectivity of the comminution process is reduced because this impingement causes comminution of the mineral matter as well as the hydrocarbonaceous material in the coal. In this connection, it has been discovered that the material discharged from the orifice at supercritical temperatures and pressures emerges from the opening in a hemispherical pattern, expanding in all directions up to 135 degrees from the direction of flow through the opening. In order to prevent any of the emerging material from impinging against the face of the orifice, the end wall or face of the orifice is preferably disposed in relation to the direction of flow through the opening so as to form an angle of about 90 degrees to about 135 degrees.

The shattered or comminuted product is preferably produced as a suspension of micron sized solid particles in vapor, i.e. steam in the case of water. This product may then be passed to various recovery units including units for the fractionation of the mineral particles from the hydrocarbonaceous particles as well as fractionating the hydrocarbonaceous particles from the vapor. For example, a cyclone can be used to fractionate the mineral fraction of the shattered coal from the hydrocarbonaceous fraction. The comminuted hydrocarbonaceous particles can be subsequently recovered using a condenser and dryer. Alternatively, the vapor phase sus-

pension may be passed directly to a burner for combustion by contact with oxygen at high temperatures.

General Description of the Principal Operating Parameters Encountered in The Preferred Embodiment of The Present Invention

Coals are commonly ranked as anthracite, bituminous, sub-bituminous, lignite or peat. Even within these classifications coals exhibit varying characteristics in relation to the geographical region or seam from which they are mined. Though it is possible to have some variation in coal seams even on a local scale, uniformity is generally evident on a regional scale. Thus, bituminous Illinois-6 coal differs appreciably from bituminous Pittsburgh-8 coal in many respects.

The characteristics of the product of the comminution process vary somewhat with the characteristics of the feed coal. For example, a bituminous coal, Illinois-6, was comminuted to a mean volumetric particle size of 3.09 microns by operation at 9200 psia and 760° F. A bituminous coal, Pittsburgh-8, was comminuted to a volumetric mean particle size of 2.96 microns by operation at 6600 psia and 800° F.

The examples and experiments described herein are representative of the results obtained for the listed types of coal. However, it is noted that in order to obtain optimum results for any particular coal supply, a certain amount of empirical studies should be made.

The more significant operating variables of the process of the invention include temperature, pressure and residence time of the slurry at supercritical conditions, together with choice of soluble additives. Various pressures and temperatures ranging from subcritical up to 1000° F. and 16,000 psia have been investigated. As indicated earlier, the mean particle size of the comminuted product is significantly reduced as the temperature and pressure of the slurry are increased from the subcritical into the supercritical range of the water while the scissioning of the hydrocarbonaceous material from the mineral material and the alcohol solubility of the hydrocarbonaceous material is significantly increased by increasing from a subcritical temperature and/or pressure to supercritical.

For example, the following table illustrates the differences obtained by conducting a continuous explosive comminution operation at subcritical conditions versus supercritical conditions. In each instance, the coal was an Illinois-6 coal having an initial particle size range of about 5 to 150 microns and a mean particle size of about 75 microns. In each run, the feed coal was mixed with sufficient water to provide a slurry containing about 20 wt % coal.

TABLE I  
SIZE DISTRIBUTION OF EXPLOSIVELY  
SHATTERED AT SUB- AND SUPERCRITICAL  
TEMPERATURE CONDITIONS

| Particle Size      | Conditions           |                      |                       |                       |
|--------------------|----------------------|----------------------|-----------------------|-----------------------|
| Range<br>(Microns) | 660° F.<br>8600 psig | 700° F.<br>5400 psig | 830° F.<br>12400 psig | 860° F.<br>10000 psig |
| 125-178            | 3.9 vol. %           | 0.0 vol. %           | 0.0 vol. %            | 0.0 vol. %            |
| 88-124.9           | 18.1                 | 4.5                  | 0.6                   | 0.0                   |
| 62-87.9            | 17.2                 | 11.5                 | 0.0                   | 0.0                   |
| 44-61.9            | 16.0                 | 12.7                 | 0.0                   | 15.4                  |
| 31-43.9            | 11.9                 | 10.2                 | 0.0                   | 0.0                   |
| 22-30.9            | 9.0                  | 13.7                 | 0.0                   | 0.0                   |
| 16-21.9            | 6.8                  | 13.6                 | 0.0                   | 0.0                   |
| 11-15.9            | 3.8                  | 9.7                  | 0.6                   | 0.0                   |
| 7.8-10.9           | 4.6                  | 7.0                  | 7.6                   | 0.0                   |
| 5.5-7.7            | 1.9                  | 5.6                  | 16.3                  | 6.8                   |

TABLE I-continued

SIZE DISTRIBUTION OF EXPLOSIVELY  
SHATTERED AT SUB- AND SUPERCRITICAL  
TEMPERATURE CONDITIONS

| Particle Size                | Conditions           |                      |                       |                       |
|------------------------------|----------------------|----------------------|-----------------------|-----------------------|
| Range<br>(Microns)           | 660° F.<br>8600 psig | 700° F.<br>5400 psig | 830° F.<br>12400 psig | 860° F.<br>10000 psig |
| 3.9-5.4                      | 2.5                  | 4.7                  | 17.1                  | 11.4                  |
| 2.8-3.8                      | 2.4                  | 3.1                  | 15.5                  | 15.4                  |
| 1.9-2.7                      | 0.8                  | 2.0                  | 27.9                  | 33.8                  |
| 1.4-1.8                      | 0.4                  | 1.0                  | 13.9                  | 16.9                  |
| Volumetric<br>Mean           |                      |                      |                       |                       |
| Particle Size,<br>15 Microns | 49.2                 | 23.6                 | 2.71                  | 3.27                  |

The results show that the volumetric mean particle size of the product produced by comminution at supercritical conditions are about an order of magnitude smaller than the volumetric mean particle size obtained by comminution at subcritical conditions. In addition, supercritical conditions provide a product wherein a substantial portion of the product has a particle size of less than about 5 microns whereas operation at subcritical conditions provides a product with only a small fraction of its particles reduced to this size range.

It has been found that by operating at subcritical conditions, the mean product particle size initially decreases linearly with respect to increasing pressure until the pressure reaches about 7,000 psia. Increasing the pressure beyond this level produces a continued decrease in particle size. The decrease, however, is not as appreciable in response to increased temperature in this range as it is in the lower pressure range. The effect of temperature on the product mean particle size is somewhat more complex than that of pressure. The mean particle size of the product initially decreases with respect to increasing temperatures up to an optimum value for the coal in the slurry. Increasing the temperature beyond that point, however, while maintaining a constant pressure, increases the mean particle size of the product.

Other variables in operation of the invention include the identity and/or properties of the feed coal, the slurry fluid, the amount of coal in the slurry, the raw feed particle size, the size of the orifice passage or opening, and the length of time required for the slurry to pass across the opening. Preferred slurries for use in the present invention utilize water or methanol as the slurry fluid and have solids contents between about 10% and about 60% by weight. The degree of comminution obtained, however, is substantially independent of solids content. The upper limit on solids content of the slurry is determined principally by the ability to pump or otherwise handle a high solids content slurry and to avoid agglomeration at the high temperatures employed in the present invention, i.e. solids handling and agglomeration problems increase as the percent solids in the slurry increases. It is preferable, however, to use as high a solids content as possible to avoid wasting energy by heating and pressuring unnecessary amounts of slurry fluid.

As used herein, the percent solids in the coal slurry is defined as follows:

$$\left( \frac{\text{grams Dry Coal}}{\text{grams Dry Coal} + \text{Liquid}} \right) \times 100 = \% \text{ Solids in slurry}$$

This calculation requires the coal to be dried to a constant weight basis at a temperature of 110° C. to make this determination. In actual practice, however, the coal is not dried before the slurry is formed. Rather, the slurry is formed from a coal on an "as-received" basis and the solids content is then determined by filtering a weighed amount of the slurry, and drying the resultant filter cake.

As indicated, the amount of solids in the slurry does not materially affect the size distribution of the final product. It is again emphasized, however, for purposes of economics, to use as high a solids content as can be reasonably pumped and heated.

In general, the maximum solids content that can be pumped by known pumping equipment is an aqueous slurry containing about 50-60% by weight coal. Coarser coal particles in the slurry permit higher solids contents; finer coal particles in the slurry require lower solids contents.

In addition, the percent solids in the feed can have some effect on the heating characteristics of the slurry relative to fouling of the heating operations. In general, higher solids contents can produce higher fouling rates during the heating operations.

As the feed particles increase in size, the necessary residence time will increase. In any event, the size of the feed particles must be smaller than the orifice opening to avoid plugging the orifice. The preferred size of the orifice opening is at least three times as large as the size of the largest feed particles. The size of the feed particles dictates pressure, temperature and residence time for each type of coal, and is best determined empirically. The size of the solids particles may thus be increased as the size of the orifice opening is increased.

The length of time desired for the slurry to cross the opening determines the length of the opening. That is, the length of the opening must be designed so that, considering the velocity of slurry through the opening, the time in crossing the opening will be less than a predetermined maximum. As explained previously, it has been discovered that this length of time should be as small as possible so that the supercritical fluid is not permitted to escape from the pores of the solid in the orifice, as opposed to instantaneously escaping in the explosion zone to disrupt the solid in less than about 10 microseconds and preferably less than about 1 microsecond.

Experimental results have been correlated to show the effect of temperature, pressure and residence time on the shattered product particle size. It is useful for present purposes to combine the effects of temperature and pressure into a single variable referred to as the net enthalpy of the water. This variable is defined as follows:

$$\text{Net Enthalpy (NE)} = \left[ \frac{\text{enthalpy of water at operating temperature and pressure}}{\text{Enthalpy Water at } 212^\circ \text{ F. and } 1 \text{ atm.}} \right] \times \frac{\text{Fraction of Water that will be Converted to Steam}}{}$$

NE is expressed as "BTU/in<sup>3</sup>". An empirical equation has been obtained to calculate the net enthalpy in the

temperature and pressure ranges of importance. The equation in terms of temperature, pressure and square of temperature is:

$$NE = 8.172(T) + 0.15022(P) - 0.38469(T^2) - 29.664$$

where:

NE is expressed as BTU/in<sup>3</sup>

T = temperature in °F.  $\times 10^{-2}$

P = pressure in psia  $\times 10^{-3}$

This equation has a correlation coefficient of 0.995 where:

$5,000 < P < 15,000$  psia

$700 < T < 900$  °F; and

$P \div [(42.5 T) - 27200] < 1$

The preferred residence time at these conditions is about 5 seconds.

The correlation of these higher temperatures and pressures on the mean product particle size of Illinois-6 coal (including its unaffected mineral matter), assuming residence time of about 5 seconds, is expressed by the following equation:

$$\log \mu = 7.7575 - 0.4742 (NE)$$

Where  $\mu$  = volumetric mean particle size in microns and net enthalpy (NE) is expressed in BTU/in<sup>3</sup> of water. Temperatures between about 800° and about 950° F. and pressures between about 7,000 and 12,000 psia consistently yielded a shattered product having a mean particle size ranging between 2.5 and 6 microns. FIG. 2 illustrates the mean particle size in microns of the shattered product of Illinois-6 feed coal as a function of the temperature and pressure conditions in the process of the invention.

The effect of high temperature and pressure on the shattering of Illinois-6 coal indicates the existence of an inverse linear relationship between the log mean volumetric particle size of the shattered product and the net enthalpy of the slurry in the shattering unit. Thus, the logarithm of the volumetric mean particle size decreases linearly in relation to increases of the net enthalpy in the comminution system.

A parametric study similar to the one with Illinois-6 coal explained above was conducted for Pittsburgh-8 coal. Correlation was obtained for mean particle size of the shattered product as a function of net enthalpy and log of net enthalpy. The equation may be expressed as follows:

$$\mu = 374.8 + 17.19 (NE) - 231.38 \ln (NE)$$

where:  $\mu$  = volumetric mean particle size in microns

NE = net enthalpy in BTU/in<sup>3</sup>.

FIG. 3 shows the volumetric mean particle size in microns of the shattered product Pittsburgh-8 coal and its mineral content as a function of temperature and pressure conditions in the process of the invention.

An investigation of the effect of the size of the feed coal on the size of the shattered product included feed coal with maximum particle sizes ranging from about 50 microns to about 240 microns. All feed sizes produced substantially similar, successful shattering results. Accordingly, it is possible to further increase the maximum shatterable feed size by the installation of orifices with larger diameter since our results indicate that mean particle size of the shattered product is substantially independent of feed size.

## Description of the Comminuted Product

The product resulting from the explosive comminution of coal according to this invention has been tested by a variety of physical and physiochemical analyses. These analyses show that the feed coal can be comminuted and then separated if desired into two distinct components or fractions. One of the fractions, a hydrocarbonaceous fraction, consists substantially of hydrocarbonaceous particles which have comminuted to a very fine particle size, i.e. less than 5 microns in diameter. This hydrocarbonaceous fraction has a lower density, a higher solubility and a different rate of oxidation in ambient atmosphere than either the original feed stock or coal comminuted at subcritical conditions. Moreover, this hydrocarbon fraction includes a subfraction of particles having a particle size of less than two microns in diameter. These particles consist essentially of hydrocarbons and are characterized by the substantially complete absence of ash forming minerals or sulfur of any form.

An analysis according to ASTM designated procedures (1977 Annual Book of ASTM Standards, Part 26) of raw feed coals and the resultant explosively shattered products were performed and the results are listed in Table II below. The explosively comminuted products were collected by quenching with water. The product analysis applies to the resultant filtered and water-washed product solids with no removal of mineral matter.

30

carbonaceous fraction of the product coal is a substantially different substance than the original coal.

## I. Mean Product Particle Size

In the data discussed below, the size distribution analysis of the product coal particles was accomplished with a laser beam scattering technique using a MICROTRAC particle size analyzer manufactured by the Leeds/Northrup Co., Inc. The MICROTRAC unit operates by measuring the scattering of light from a laser beam in a defined field and calculating the volume of each counted particle within that defined field, assuming all particles to be spherical. The particles are sorted into a predetermined range of volume sizes and the percentage of total particles within each volume size range is determined. The results are converted to mean particle diameters and listed as a percentage of particles having a volumetric mean particle diameter within a defined mean particle diameter range.

The volume distribution method of calculating mean particle size is a method of statistically weighting the reported mean particle diameter to avoid favoring the more numerous, smaller particles and to approximate the size distribution on a weight basis. For example, when a comminuted product is analyzed first by the direct count method and then by the volume distribution method, as reported in Table III, the direct count method reports a smaller mean particle size than is reported by the volume distribution used therein.

TABLE II

PROXIMATE AND ULTIMATE ANALYSIS OF FEED  
AND EXPLOSIVELY SHATTERED PRODUCT

|                                 | Illinois-6 |         | Pittsburgh-8 |         |
|---------------------------------|------------|---------|--------------|---------|
|                                 | FEED       | PRODUCT | FEED         | PRODUCT |
| <u>PROXIMATE ANALYSIS, WT %</u> |            |         |              |         |
| % Volatile                      | 36.85      | 32.27   | 31.49        | 30.59   |
| Btu/lb                          | 11,206     | 11,504  | 13,449       | 13,140  |
| % Fixed Carbon                  | 44.07      | 48.53   | 57.71        | 58.89   |
| <u>ULTIMATE ANALYSIS, WT %</u>  |            |         |              |         |
| Carbon                          | 63.22      | 64.98   | 74.67        | 73.90   |
| Hydrogen                        | 4.49       | 4.13    | 4.76         | 4.77    |
| Nitrogen                        | 1.19       | 1.02    | 1.27         | 1.46    |
| Chlorine                        | 0.20       | 0.03    | 0.05         | 0.03    |
| Sulfur                          | 4.79 {     | 3.80 {  | 2.25 {       | 2.15 {  |
| Sulfate                         | 0.19       | 0.03    | 0.00         | 0.00    |
| Pyritic                         | 2.25       | 1.57    | 1.27         | 1.00    |
| Organic                         | 2.35       | 2.20    | 0.98         | 1.15    |
| Ash                             | 19.08      | 19.10   | 10.80        | 10.52   |
| Oxygen (Diff.)                  | 7.03       | 6.94    | 6.20         | 7.17    |
| TOTAL                           | 100.00     | 100.00  | 100.00       | 100.00  |
| <u>ASH ANALYSIS, WT %</u>       |            |         |              |         |
| SiO <sub>2</sub>                | 50.83      | 53.89   | 55.65        | 52.64   |
| Al <sub>2</sub> O <sub>3</sub>  | 19.19      | 19.11   | 23.86        | 23.18   |
| TiO <sub>2</sub>                | 0.81       | 0.92    | 1.10         | 1.10    |
| Fe <sub>2</sub> O <sub>3</sub>  | 16.64      | 17.66   | 14.01        | 17.96   |
| CaO                             | 4.80       | 3.95    | 0.70         | 0.97    |
| MgO                             | 1.05       | 1.05    | 0.66         | 0.75    |
| K <sub>2</sub> O                | 1.87       | 1.85    | 1.70         | 1.50    |
| Na <sub>2</sub> O               | 1.25       | 0.40    | 0.43         | 0.42    |
| SO <sub>3</sub>                 | 3.16       | 0.99    | 0.65         | 0.91    |
| P <sub>2</sub> O <sub>5</sub>   | 0.15       | 0.15    | 0.31         | 0.25    |
| Undetermined                    | 0.25       | 0.03    | 0.93         | 0.32    |
| TOTAL                           | 100.00     | 100.00  | 100.00       | 100.00  |

These results show that the overall composition of the coal is not significantly altered within the range of experimental error by the practice of the present invention. Yet, as the following experiments show, the hydro-

65

TABLE III

COMPARISON OF REPORTED RESULTS  
Volume Distribution Basis vs. Direct Count Basis

| Particle Diameter Range (Microns) | Direct Count of Product Particles Within Range (%) | Volume of Particles Within Range (%) | Accumulated particle count, (%) <sup>1</sup> | Accumulated Volume, (%) <sup>2</sup> |
|-----------------------------------|----------------------------------------------------|--------------------------------------|----------------------------------------------|--------------------------------------|
| 178-125                           | 0.0                                                | 0.0                                  | 100.0                                        | 100.0                                |
| 125-88                            | 0.0005                                             | 3.4                                  | 99.999                                       | 96.6                                 |
| 88-62                             | 0.0021                                             | 4.9                                  | 99.997                                       | 91.7                                 |
| 62-44                             | 0.0151                                             | 12.3                                 | 99.98                                        | 79.4                                 |
| 44-31                             | 0.0490                                             | 14.1                                 | 99.93                                        | 65.3                                 |
| 31-22                             | 0.1267                                             | 12.9                                 | 99.81                                        | 52.4                                 |
| 22-16                             | 0.4284                                             | 16.3                                 | 99.38                                        | 36.1                                 |
| 16-11                             | 0.8611                                             | 11.6                                 | 98.52                                        | 24.5                                 |
| 11-7.8                            | 1.8672                                             | 8.6                                  | 96.65                                        | 15.9                                 |
| 7.8-5.5                           | 3.6884                                             | 5.8                                  | 92.96                                        | 10.1                                 |
| 5.5-3.9                           | 7.5353                                             | 4.2                                  | 85.43                                        | 5.9                                  |
| 3.9-2.8                           | 14.0921                                            | 2.9                                  | 72.33                                        | 3.0                                  |
| 2.8-1.9                           | 28.7044                                            | 2.0                                  | 42.63                                        | 1.0                                  |
| 1.9-1.4                           | 42.6297                                            | 1.0                                  | 0.00                                         | 0.0                                  |

## Mean Particle Size

By Direct Count: 2.13 microns

By Volume Distribution: 20.8 microns

<sup>1</sup>Accumulated number of product particles within or smaller than range (%).<sup>2</sup>Accumulated volume of particles within or smaller than range (%).

In Table III, the product analyzed by the direct count reported a mean particle size of about 2.13 microns, but the same product analyzed by the volume distribution reported a mean particle size of 20.8 microns. Importantly, although about 40% of the product particles are smaller than 2 microns, reported on a direct count basis, that 40% represents only about 1% of the mass of shattered product.

The size distribution bias, which occurs with the direct count basis, is substantially avoided when the results are reported on a volume distribution. This distinction must be appreciated when comparing the results herein with those of the prior art: a product reported herein with a volumetric mean particle diameter of about 5 microns is very substantially smaller than a product reported as having a mean particle diameter of 5 microns calculated on the direct count basis, as illustrated in columns 2 and 3 of Table III.

## SPECIFIC EXAMPLES

The advantages of the preferred embodiment of the present invention are illustrated by reference to the following examples.

## EXAMPLE I

Raw Illinois-6 coal containing 20% by weight mineral matter was pulverized by grinding the coal, passing the resultant ground coal through a 100 mesh screen, recovering the smaller than 100 mesh fraction and recycling the larger fraction back to the grinding operation. The pulverized raw coal was mixed with water to prepare a slurry of about ten (10) percent solids by weight. The slurry was pressurized and heated to supercritical conditions using methods previously described. The slurry was maintained at about 11,400 psia and about 810° F. for at least 5 seconds after which the slurry was then passed through an adiabatic expansion orifice into an expansion zone maintained at a temperature of 212° F. and pressure of 14.5 psia within about 0.3 microsecond. The size distribution of the feed and of the resultant shattered product with all minerals present and essentially unchanged in size are listed in Table IV.

TABLE IV

## SIZE DISTRIBUTION OF FEED AND EXPLOSIVELY SHATTERED PRODUCT OF ILLINOIS-6 COAL

| Particle Size Range (Microns) | Volume Percent |                     | Hydrocarbonaceous Portion of Product |
|-------------------------------|----------------|---------------------|--------------------------------------|
|                               | Feed           | Total Product       |                                      |
| 125-178                       | 12.9           | 2.3                 | 2.4                                  |
| 88-124.9                      | 20.7           | 1.1                 | 1.3                                  |
| 62-87.9                       | 18.6           | 0.0                 | 0.0                                  |
| 44-61.9                       | 19.7           | 0.0                 | 0.0                                  |
| 31-43.9                       | 7.0            | 0.0                 | 0.0                                  |
| 22-30.9                       | 3.7            | 0.0                 | 0.0                                  |
| 16-21.9                       | 6.1            | 0.0                 | 0.0                                  |
| 11-15.9                       | 4.2            | 0.0                 | 0.0                                  |
| 7.8-10.9                      | 1.3            | 6.0                 | 4.0                                  |
| 5.5-7.7                       | 0.9            | 14.8                | 14.4                                 |
| 3.9-5.4                       | 2.0            | 15.7                | 15.1                                 |
| 2.8-3.8                       | 1.9            | 15.0                | 14.7                                 |
| 1.9-2.7                       | 0.1            | 29.8                | 32.1                                 |
| 1.4-1.8                       | 0.0            | 14.9                | 16.0                                 |
| Mean Particle Size (Microns)  | 64.9           | 3.09 <sup>(a)</sup> | 2.84                                 |

<sup>(a)</sup>Includes mineral particles with unchanged particle size distribution.

Next, samples of the product and raw feed coal were subjected to a low-temperature ashing using activated oxygen plasma. This removed all hydrocarbon from the mineral component, which was left substantially in its natural state and analyzed for size distribution. The results are set forth in Table V.

TABLE V

## MINERAL PARTICLE SIZE DISTRIBUTION IN FEED AND EXPLOSIVELY SHATTERED PRODUCT OF ILLINOIS-6 COAL

| Particle Size Range (Microns) | Volume Percent |         |
|-------------------------------|----------------|---------|
|                               | Feed           | Product |
| 125-178                       | 0.0            | 0.5     |
| 88-124.9                      | 0.8            | 0.2     |
| 62-87.9                       | 3.2            | 0.0     |
| 44-61.9                       | 6.5            | 3.6     |
| 31-43.9                       | 2.9            | 5.1     |
| 22-30.9                       | 5.0            | 7.4     |
| 16-21.9                       | 9.2            | 8.4     |
| 11-15.9                       | 10.7           | 11.2    |
| 7.8-10.9                      | 15.2           | 12.6    |
| 5.5-7.7                       | 13.9           | 11.7    |
| 3.9-5.4                       | 12.8           | 13.0    |
| 2.8-3.8                       | 8.2            | 11.0    |
| 1.9-2.7                       | 6.7            | 9.7     |
| 1.4-1.8                       | 3.3            | 4.8     |
| Mean Particle Size (Microns)  | 8.48           | 7.36    |

The results show that the mean particle size of the minerals contained in the feed coal remains substantially unaffected by the explosive comminution process whereas the particle size of the feed, as a whole, is greatly reduced by the shattering operation. In other words, substantially all of the explosive shattering force results in reducing the mean particle size of the hydrocarbon in the feed coal and not of the undesired ash forming or mineral portion of the coal. Moreover, since the minerals exhibit a larger particle size, many of the particles of the final product in the larger size range can be attributed to the minerals and that the mean particle size of the hydrocarbon in the overall product as indicated is less than the mean particle size observed for the product overall.

## EXAMPLE II

Example I was repeated using a Pittsburgh-8 coal containing 10 percent mineral matter. The effect of the explosive comminution reaction on the mean particle

size of the feed and of the mineral component of the feed are set forth below in Tables VI and VII, respectively.

TABLE VI

| SIZE DISTRIBUTION OF FEED AND EXPLOSIVELY SHATTERED PRODUCT OF PITTSBURGH-8 COAL |                |                     |                                      |
|----------------------------------------------------------------------------------|----------------|---------------------|--------------------------------------|
| Particle Size Range (Microns)                                                    | Volume Percent |                     | Hydrocarbonaceous Portion of Product |
|                                                                                  | Feed           | Total Product       |                                      |
| 125-178                                                                          | 8.0            | 0.0                 | 0.0                                  |
| 88-124.9                                                                         | 11.9           | 0.0                 | 0.0                                  |
| 62-87.9                                                                          | 28.5           | 0.0                 | 0.0                                  |
| 44-61.9                                                                          | 19.9           | 2.6                 | 3.0                                  |
| 31-43.9                                                                          | 7.7            | 1.6                 | 1.8                                  |
| 22-30.9                                                                          | 7.4            | 0.0                 | 0.0                                  |
| 16-21.9                                                                          | 4.4            | 0.0                 | 0.0                                  |
| 11-15.9                                                                          | 6.2            | 5.5                 | 5.3                                  |
| 7.8-10.9                                                                         | 3.0            | 3.4                 | 2.3                                  |
| 5.5-7.7                                                                          | 0.0            | 3.4                 | 1.0                                  |
| 3.9-5.4                                                                          | 1.0            | 20.9                | 22.0                                 |
| 2.8-3.8                                                                          | 1.5            | 21.2                | 22.7                                 |
| 1.9-2.7                                                                          | 0.0            | 25.4                | 27.3                                 |
| 1.4-1.8                                                                          | 0.0            | 12.7                | 13.7                                 |
| Mean Particle Size (Microns)                                                     | 60.50          | 3.32 <sup>(a)</sup> | 3.02                                 |

<sup>(a)</sup>Includes mineral particles with unchanged particle size distribution.

TABLE VII

| MINERAL PARTICLE SIZE DISTRIBUTION IN FEED AND EXPLOSIVELY SHATTERED PRODUCT OF PITTSBURGH-8 COAL |                |         |
|---------------------------------------------------------------------------------------------------|----------------|---------|
| Particle Size Range (Microns)                                                                     | Volume Percent |         |
|                                                                                                   | Feed           | Product |
| 125-178                                                                                           | 0.0            | 0.0     |
| 88-124.9                                                                                          | 2.5            | 0.0     |
| 62-87.9                                                                                           | 1.2            | 0.0     |
| 44-61.9                                                                                           | 0.3            | 0.0     |
| 31-43.9                                                                                           | 1.4            | 0.0     |
| 22-30.9                                                                                           | 0.7            | 1.2     |
| 16-21.9                                                                                           | 5.1            | 3.8     |
| 11-15.9                                                                                           | 9.1            | 9.0     |
| 7.8-10.9                                                                                          | 14.0           | 14.1    |
| 5.5-7.7                                                                                           | 15.4           | 17.0    |
| 3.9-5.4                                                                                           | 15.8           | 17.3    |
| 2.8-3.8                                                                                           | 12.9           | 13.8    |
| 1.9-2.7                                                                                           | 13.9           | 15.6    |
| 1.4-1.8                                                                                           | 6.9            | 7.8     |
| Mean Particle Size                                                                                | 5.50           | 4.98    |

These results closely parallel the results previously observed for Illinois-6 coal and show that explosive comminution technique, as taught by this invention, results in a great selectivity of comminution. Whereas the total feed coal is reduced from a mean particle size of about 60 microns to about 3 microns, the mineral content is substantially unaffected, its mean particle size being reduced by only about 1 micron or less.

## II. Density of Product

The density<sup>1</sup> of the feed coal is greatly changed through utilization of the method of this invention. A typical raw feed coal has a density of approximately 1.3 to 1.4 g/cc. The

<sup>1</sup> As used herein, density refers to the apparent density of the individual particles, hydrocarbon fraction of the shattered product produced in accordance with this invention, by way of contrast, is about 50% to 75% of the density of the feed coal, specifically an apparent density of about 0.7 to about 0.9 g/cc. This difference cannot be accounted for by mineral constituents. No known raw coal or presently identified hydrocarbon fraction of raw coal has a density as low as that of the hydrocarbon fraction of the explosively shattered product obtained by the present invention. Similarly, the product explosively shattered at supercritical conditions has a density less than that produced by explosive shattering or comminution at subcritical temperatures and pressures. The low density of the hydrocarbon fraction makes this substance particularly useful for producing stable suspensions of the shattered coal in petroleum fuels and as a result may be used to extend this fuel.

The manner in which the invention changes the density of the coal hydrocarbon fraction is not presently fully understood. It seems likely that the invention has resulted in expansion of the pores of the hydrocarbon, and an increase in the amount of gases entrapped within the coal. Gaseous displacement tests have shown that relatively large amounts of carbon dioxide are trapped within the hydrocarbon fraction. These tests involve passing a stream of oxygen or nitrogen through a slurry of the hydrocarbon fraction and collecting and analyzing the gas stripped from the slurry. The tests show that either oxygen or nitrogen displaces about the same but significant quantity of carbon dioxide. It is possible that carbon dioxide is formed by chemical interaction of coal and water during the explosive shattering operation and the CO<sub>2</sub> is trapped within the pores of the hydrocarbon fraction.

The density of the various minerals, by way of contrast, lies from about 2 to about 5 g/cc. This density is substantially unchanged by the explosive comminution process. Since the minerals are from about 3 to about 7 times more dense than the fine coal and since the hydrocarbonaceous fraction has smaller mean particle size than that of the minerals, the hydrocarbonaceous fraction can be separated from the minerals by gravitational methods and apparatus well known to those trained in the art such as a cyclone. For example, a cyclone can separate a hydrocarbon fraction having a particle size of about 5 microns in diameter from ash and minerals having a particle size of about 3 microns in diameter because of the respective differences in mass.

## III. Solubility of Product

Solubility tests show a further change in the product brought about by the process of the present invention. Raw feed coal is soluble in organic solvents to a slight extent, generally ranging from about 0.5 to about 5 percent depending upon the type of coal and solvent. It was not expected that the process of the present invention would significantly change the solubility of the shattered coal product. It was further discovered, however, that the solubility of the comminuted product is higher with respect to many known solvents than the solubility of the feed coal, ball-milled feed coal of comparable size, coal explosively shattered at subcritical temperatures and pressures or of any known form of coal.

In mechanical stirring solubility tests, a pre-weighed and dried sample of coal was placed in a beaker along with a measured volume of solvent (typically 250 ml). The beaker was then covered and the mixture stirred with a magnetic stirrer. The stirring was stopped the following day and the coal solubility determined by one of two methods. For the diluted mixtures, i.e., where the pre-weighed sample was less than about 5 grams, the mixture was simply filtered and the undissolved coal was dried and weighed. The weight of the dissolved coal was calculated by subtracting the weight of the undissolved coal from that of the original weight of coal. If the mixture was more concentrated, i.e., where the pre-weighed sample was more than about 25 grams, a large sample was removed and centrifuged. The clear solution was then decanted. After measuring its volume, the decanted solution was evaporated and the residual coal weighed. From the weight of this residual coal and the volume of the decanted solution, the solubility of the coal could be calculated.

The increase in solubility of the shattered product versus the feed coal has been shown in connection with solvents including carbon tetrachloride, gasoline, benzene, methanol and Tetralin. The results are set forth in Table VIII below. As a control, solubilities were also determined for the raw feed coal and for the raw feed coal which had been ball milled to approximately the same particle size as the shattered product. The results indicate that the unexpected increase in solubility of the shattered product is not simply a function of size reduction or particle size. To the contrary, ball milling generally reduced the solubility of the coal.

TABLE VIII

| Sample                       | SOLUBILITY OF EXPLOSIVE SHATTERED,<br>BALL-MILLED ULTRAFINE AND FEED COALS<br>IN VARIOUS ORGANIC SOLVENTS<br>UNDER AMBIENT CONDITIONS |                    |                |          |       |
|------------------------------|---------------------------------------------------------------------------------------------------------------------------------------|--------------------|----------------|----------|-------|
|                              | Gasoline                                                                                                                              | Fraction Soluble % | Carbon         |          |       |
|                              | Benzene                                                                                                                               | Methanol           | Tetra-chloride | Tetralin |       |
| <b>Explosively Shattered</b> |                                                                                                                                       |                    |                |          |       |
| Pittsburgh-8                 | 8.85                                                                                                                                  | 10.66              | 12.96          | 5.19     | 11.35 |
| Illinois-6                   | 6.29                                                                                                                                  | 7.85               | 16.97          | 20.90    | 3.28  |
| <b>Ball Milled</b>           |                                                                                                                                       |                    |                |          |       |
| Pittsburgh-8                 | 0.48                                                                                                                                  | 2.30               | 2.09           | 0.97     | 0.87  |
| Illinois-6                   | 0.37                                                                                                                                  | 1.55               | 2.65           | 0.44     | 0.98  |
| <b>Feed</b>                  |                                                                                                                                       |                    |                |          |       |
| Pittsburgh-8                 | 1.50                                                                                                                                  | 1.92               | 2.67           | 4.88     | 1.82  |
| Illinois-6                   | 0.85                                                                                                                                  | 3.08               | 1.70           | 3.85     | 2.53  |

A comparison of the results contained in Table VIII shows that the solubility of the shattered product is about 2 to about 6 times greater than the solubility of the feed coal and about 3 to about 18 times greater than the solubility of similarly sized feed coal prepared by ball milling.

The increase in solubility of the shattered product is further confirmed by experiments using methanol extracts of the shattered product, the feed coal, and feed coal ball milled to a particle size comparable to that of the shattered product. The results, shown in FIGS. 9 and 10 for Illinois-6 and Pittsburgh-8 coals, respectively, illustrate the absorbence of the extracts of various coals by methanol as against time. The samples were analyzed on a Water Model 244 ALC/GPC liquid chromatograph equipped with a Model 660 Solvent Programmer for gradient elution and a Schaeffel HS870 UV - visible detector. Elution on a 4 mm × 30 cmu bondpak C18 column was achieved by a methanol water gradient going from 60% methanol to 100% methanol in 20 minutes. The samples were monitored for aromatic components at 254 nm.

It is noted by way of interpretation of FIGS. 9 and 10, that the initial sharp peak at 1 minute is due to aromatics derived from the raw coal rather than the solubility of the solid hydrocarbon component. These aromatics have been removed from the shattered product during the shattering and recovery process and, thus, these peaks should be ignored for purposes of comparison. Second, the discontinued section in the graph of Illinois-6 coal (FIG. 9) occurs because the solubility of this coal exceeded the scale of the recorder. Third, solubilities of the different coals varies with different solvents. The solubility, for example, of Pittsburgh-8 coal in methanol is not as great as that of Illinois-6 coal. However, the results of both experiments confirm the earlier results of the mechanical stirring experiments.

The increase in solubility occurs to a significant degree only when operating at supercritical conditions, a fact which further confirms the importance of operating at supercritical conditions. For example, referring to Table I, the product comminuted at 700° F. and 5400 psia had a solubility in methanol of only 7.29% whereas the product of the same feed exploded at 830° F. and 12,400 psia has a solubility of 19.60%. In general, the product exploded at supercritical temperatures and pressures has a methanol solubility of at least about two times greater than produced by exploding the same feed coal at subcritical temperatures and/or pressures.

#### IV. Reactivity of Explosively Shattered Coal

15 The reactivity of the shattered product and of the feed coals was compared by evaluating their respective oxidation rates, determined using thermogravimetric analysis in air at a constant rate of heating of about 40° C./minute. The thermograms of the shattered product and of the feed coal using an Illinois-6 and a Pittsburgh-8 coals are shown in FIGS. 7 and 8, respectively.

20 The explosively shattered products of the Illinois-6 and of the Pittsburgh-8 coal show the presence of a low-temperature combustible constituent which starts reacting at about 280° C. and peaks at about 300° C.

25 This low temperature combustible component is not present in known coal hydrocarbons. The low temperature peak of the shattered product is a true oxidation reaction rather than a volatilizing of components in the coal, as was shown by the fact that the peak is not present when the experiment was repeated in a nitrogen atmosphere. Thermograms of conventional coals exhibit a low-temperature peak at 100° C. which is attributable to the volatilization of water. Since the water and volatile materials are not present in the dried shattered product of this invention, the low temperature peak of conventional coal thermograms should not be considered for comparative purposes. Decomposition of the low temperature combustible component was recorded to be complete at about 350° C.

30 Peak oxidation temperature refers to the temperature at which the coal exhibits its highest rate of weight loss. The peak oxidation temperature of conventional coals generally increases with the rank of the coal. The shattered product sample had a lower peak oxidation temperature than that of the feed coals and of other comparably ranked known coal forms. For example, the peak

35 oxidation temperature of the shattered product of bituminous coal, Illinois-6, is reduced to that of the more reactive sub-bituminous ranks of coal. The rate of oxidation, or rate of weight loss, of the shattered bituminous coal at lower temperatures is also as great or greater than that of the sub-bituminous coals, as shown by the FIGS. 7 and 8. However, the heating value of the shattered bituminous rank coals, remained relatively unchanged from the heating value of the feed coal. For example, the heating value of the Illinois-6 feed coal was 11,206 BTU/lb. and of the shattered product, 11,504 BTU/lb. The Pittsburgh-8 feed coal had a heating value of 13,449 BTU/lb. and the shattered product, 13,410 BTU/lb.

#### V. Fractionation of Product

65 As indicated earlier, the amount of mineral matter contained in coal varies with the source of the coal. In general, the process of the present invention is applicable for mineral removal from coals containing greater than about 5% by weight mineral matter although the

process can be used for coal containing lesser amounts of mineral matter where economically feasible, and a finely divided product is desired. Particularly advantageous results are obtained with coals containing about 5-30 wt % mineral matter. Particularly preferred are coals containing about 7-25% mineral matter. In addition, the present invention can be utilized with coke and char materials containing up to about 40-60% by weight mineral matter.

According to a preferred embodiment of the present invention, porous hydrocarbonaceous materials such as coal are comminuted and then fractionated into at least one hydrocarbonaceous enriched fraction and at least one mineral enriched fraction. The exact degree of fractionation that can be obtained is, in general, dependent upon the source of the coal and the amount and particle size distribution of mineral matter contained in the coal. By use of the term "hydrocarbonaceous enriched fraction" is meant that more than about 50 wt % of the mineral matter originally present in the coal has been removed from the original material. Accordingly, the hydrocarbonaceous fraction contains less than about 50 wt % of the mineral matter originally present in the coal. Particularly preferred are hydrocarbonaceous fractions containing less than 75% of the mineral material originally present in the coal.

Similarly, the term "mineral enriched fraction" means that more than 50% of the mineral material originally present in the coal is contained in the mineral fraction. Preferably more than 75% of the mineral material originally present in the coal is contained in the mineral fraction. Particularly preferred are enriched mineral fractions containing more than 85% of the mineral material originally present in the coal.

#### VI. Clean Coal Subfraction

As previously mentioned, all known raw coals contain some degree of sulfur in organic form and inorganic forms, e.g., pyrites and sulfates. It was unexpected to find that the explosive comminution technique of the invention had removed the organic sulfur from at least a portion or subfraction, referred to herein as a "clean coal" component or subfraction of the hydrocarbon fraction of the shattered product. The clean coal component consists of that portion of the hydrocarbonaceous fraction having a particle size of less than about 2 microns.

Studies were conducted using electron microscopes and elemental analysis techniques to confirm the composition of these particles. Although larger particles contain small amounts of organic sulfur and mineral matter, the less than two micron sized particles are pure hydrocarbon containing no minerals or sulfur of any form. This result has been shown to occur with both Illinois-6 coal and with Pittsburgh-8 coal.

The mechanism by which this clean hydrocarbon fraction results is not fully understood. It is likely to be related to the kinetic and/or stoichiometric relation which exists between the hydrocarbon, supercritical water, the minerals and the sulfur particles at the extremely high energy and short lived conditions across the expansion unit of the reactor. This result is not attributable simply to size reduction, as shown by the fact that the removal of organic sulfur does not occur with ball milled coal, regardless of particle size.

The precise chemical and structural nature of the shattered product are not known. It is known, as shown by these chemical and physiochemical results set forth

above, that the shattered product and specifically the hydrocarbon fraction of the shattered product embody a form of coal previously unknown. The solubility, the oxidation rate, the density and the complete absence of organic sulfur show that the shattered hydrocarbon product is different from known coals and from coals conventionally ground to equivalent particle size.

#### Scissionability and Separability Studies

Two samples of totally condensed, explosively shattered product were produced and collected. The first sample was produced by the continuous heating and explosive expansion of an aqueous slurry of Illinois-6 coal from the supercritical conditions of 6400 psi and 830° F. to ambient conditions. All of the resultant product was collected and condensed. The second sample represented the continuous explosive shattering of Illinois-6 coal from the subcritical conditions of 2200 psi and 570° F.

The size distribution of the feed and each of the resultant products are set forth in Tables IX, X, and XI below.

TABLE IX

| VOLUME SIZE DISTRIBUTION OF FEED |                   |
|----------------------------------|-------------------|
| Size Range<br>μm                 | Volume<br>Percent |
| 178-125                          | 0.0               |
| 125-88                           | 16.5              |
| 88-62                            | 17.9              |
| 62-44                            | 16.4              |
| 44-31                            | 11.1              |
| 31-22                            | 8.9               |
| 22-16                            | 8.2               |
| 16-11                            | 5.8               |
| 11-7.8                           | 0.0               |
| 7.8-5.5                          | 3.1               |
| 5.5-3.9                          | 6.4               |
| 3.9-2.8                          | 2.9               |
| 2.8-1.9                          | 1.5               |
| 1.9-1.4                          | 0.7               |

Mean particle size = 44.7 μm

TABLE X

| VOLUMETRIC SIZE DISTRIBUTION OF<br>PRODUCT SAMPLE - SUB-CRITICAL<br>CONDITIONS - 570° F., 2200 psi |                   |
|----------------------------------------------------------------------------------------------------|-------------------|
| Size Range<br>μm                                                                                   | Volume<br>Percent |
| 178-125                                                                                            | 0.0               |
| 125-88                                                                                             | 13.6              |
| 88-62                                                                                              | 16.6              |
| 62-44                                                                                              | 14.7              |
| 44-31                                                                                              | 10.3              |
| 31-22                                                                                              | 9.8               |
| 22-16                                                                                              | 8.6               |
| 16-11                                                                                              | 8.7               |
| 11-7.8                                                                                             | 1.0               |
| 7.8-5.5                                                                                            | 3.1               |
| 5.5-3.9                                                                                            | 7.0               |
| 3.9-2.8                                                                                            | 3.3               |
| 2.8-1.9                                                                                            | 1.8               |
| 1.9-1.4                                                                                            | 0.9               |

Mean particle size = 36.9 μm

TABLE XI

| VOLUMETRIC SIZE DISTRIBUTION OF<br>PRODUCT SAMPLE - SUPER-CRITICAL<br>CONDITIONS - 830° F., 6400 psi |                   |
|------------------------------------------------------------------------------------------------------|-------------------|
| Size Range<br>μm                                                                                     | Volume<br>Percent |
| 178-125                                                                                              | 0.0               |
| 125-88                                                                                               | 0.0               |

TABLE XI-continued

| VOLUMETRIC SIZE DISTRIBUTION OF PRODUCT SAMPLE - SUPER-CRITICAL CONDITIONS - 830° F., 6400 psi |                   |
|------------------------------------------------------------------------------------------------|-------------------|
| Size Range<br>μm                                                                               | Volume<br>Percent |
| 88-62                                                                                          | 0.0               |
| 62-44                                                                                          | 0.0               |
| 44-31                                                                                          | 0.0               |
| 31-22                                                                                          | 0.0               |
| 22-16                                                                                          | 0.0               |
| 16-11                                                                                          | 11.3              |
| 11-7.8                                                                                         | 0.0               |
| 7.8-5.5                                                                                        | 5.3               |
| 5.5-3.9                                                                                        | 33.0              |
| 3.9-2.8                                                                                        | 20.3              |
| 2.8-1.9                                                                                        | 19.9              |
| 1.9-1.4                                                                                        | 9.9               |

Mean particle size = 3.84 μm

In addition, portions of each of the product samples collected were centrifuged to remove excess water. The resultant concentrated portions were then examined under a microscope. The microscopical particle properties of transparency, color reflectance, refractive index, birefringence, pleochroism, fluorescence, size, shape, surface texture, magnetism, solubility, melting point and density were, to the extent possible, observed. It was observed that the samples produced by subcritical conditions were of large particle size as evidenced by the data in Table X. In addition, these particles showed an appreciable number of unscissioned mineral and hydrocarbonaceous particles. Substantially all of the particles produced by supercritical conditions were small in size (Table XI) and the mineral and hydrocarbonaceous particles were scissioned.

The remaining portion of the supercritical product sample was allowed to stand for 3-4 weeks to permit the sample to gravity settle. Two distinct, upper and lower layers were produced, separated and analyzed. The results obtained are set forth in Table XII below. This data further illustrates the scissioning and separation of the mineral and hydrocarbonaceous material that was obtained by subjecting the coal to explosive comminution at supercritical conditions.

TABLE XII

ASH ANALYSIS AND X-RAY DIFFRACTION RESULTS - EXPLOSIVELY SHATTERED PRODUCT

|                                                   |         | Explosively<br>Shattered<br>Product | Upper<br>Layer | Lower<br>Layer |
|---------------------------------------------------|---------|-------------------------------------|----------------|----------------|
| Approximate<br>Relative Percent                   | Percent |                                     |                |                |
| Ash                                               |         | 13.2                                | 8.6            | 25.9           |
| Crystalline Material<br>in Ash                    |         | 61.1                                | 65.0           | 65.0           |
| Quartz                                            |         | 18.4                                | 18.3           | 16.6           |
| Fe <sub>2</sub> O <sub>3</sub>                    |         | 12.6                                | 13.3           | 13.3           |
| FeS <sub>2</sub>                                  |         |                                     |                |                |
| Ca <sub>12</sub> Al <sub>14</sub> O <sub>33</sub> |         |                                     |                |                |
| Clay                                              |         | 7.7                                 | 3.3            | 5.0            |

## COMPARATIVE EXAMPLES

The preceding data was obtained from a continuous flow pilot plant wherein a coal water slurry is directly heated by an electric current passing through the slurry, i.e. the slurry acts as a resistance heater. This apparatus cannot be utilized, however, for all possible combinations of temperature and pressure. For example, the slurry resistance heater cannot be used to heat a slurry to a high temperature unless the pressure imposed upon the system is sufficient to maintain the water in a liquid or supercritical state. In other words, the continuous flow pilot plant cannot adequately generate a superheated steam system.

Accordingly, a test procedure was developed to determine whether it was possible to accurately predict, from data obtained in the prior art superpressured water and superheated steam regimes, the results obtained by applicants when operating at supercritical pressures and temperatures. The test procedure is initiated by placing a slurry of coal and water of known weight, volume and solids content in a thin walled, open topped copper container. The container is then inserted into a circular opening, sized to receive the container, in a metal block maintained at a predetermined high temperature. The sample is then sealed within the cavity by placing a metallic seal over the opening in the block. Convection and radiation from the metallic block function to heat the sample within the copper container. Sample temperature, sample pressure and block temperature are monitored. The seal is then ruptured, on demand, by contact with a circular cutting device, at a predetermined time, temperature or pressure. When ruptured, the sample instantaneously expands or explodes from the cavity into a collection chamber. The resultant product is condensed and quantitatively recovered and analyzed.

The feed coal utilized in each of these tests is an Illinois-6 coal having an average particle size of 50.6 micrometers. The coal was added to the container as a slurry of 20 wt. % coal in water.

The specific temperatures and pressures obtained by placing the coal water slurry for predetermined time periods in a metal block maintained at a temperature of about 1000° F., 1200° F. and 1400° F. and the mean particle size of the final exploded or comminuted product are set forth in Tables XIII, XIV and XV below. In addition, each of the specific temperature and pressure conditions tested and the relationship of the conditions to the thermodynamic regimes of supercritical, superpressured water and superheated steam are graphically represented in FIG. 11.

TABLE XIII

| Wt. set, gms | Identification    | Value      | 1000° F. Block Temperature |      |      |      |     |
|--------------|-------------------|------------|----------------------------|------|------|------|-----|
|              |                   |            | 1                          | 2    | 3    | 5    | 7   |
| 4            | Run Number        | 99         | 85                         | 93   | 109  | 98   |     |
|              | Pressure, psig    | 412        | 504                        | 1200 | 1332 | 1256 |     |
|              | Sample Temp., °F. | 345        | 513                        | 677  | 662  | 628  |     |
|              | Block Temp., °F.  | 1006       | 1038                       | 1053 | 1000 | 1003 |     |
|              | Sample Wt., gm    | 4.34       | 4.01                       | 4.04 | 3.82 | 4.13 |     |
|              | Mean Size, μm     | 19.8       | 30.4                       | 27.6 | 24.1 | 21.0 |     |
| 6            | Run Number        | Insignifi- | 86                         | 94   | 100* | 102* | 101 |

TABLE XIII-continued

|              |                    | 1000° F. Block Temperature |       |       |       |       |       |
|--------------|--------------------|----------------------------|-------|-------|-------|-------|-------|
| Wt. set, gms | Value              | Time Set, Minutes          |       |       |       |       |       |
|              |                    | 1                          | 2     | 3     | 5     | 7     |       |
| 8            | Pressure, psig     | cant                       | 800   | 1392  | 1952  | 2284  | 2208  |
|              | Sample Temp., °F.  | Tempera-<br>ture           | 431   | 572   | 694   | 750   | 710   |
|              | Block Temp., °F.   | 989                        | 1000  | 1000  | 1013  | 985   |       |
|              | Sample Wt., gm     | Dif-<br>ferences           | 6.01  | 6.01  | 6.10  | 6.24  | 6.07  |
|              | Mean Size, $\mu$ m |                            | 31.4  | 27.1  | 24.3  | 23.4  | 22.3  |
|              | Run Number         |                            | 87    | 95    | 104   | 103   |       |
|              | Pressure, psig     |                            | 568   | 1560  | 3000  | 3176  |       |
|              | Sample Temp., °F.  |                            | 386   | 520   | 705   | 708   |       |
| 10           | Block Temp., °F.   |                            | 1011  | 1004  | 987   | 985   |       |
|              | Sample Wt., gm     |                            | 8.02  | 8.02  | 8.19  | 8.08  |       |
|              | Mean Size, $\mu$ m |                            | 35.8  | 30.1  | 23.0  | 22.3  |       |
|              | Run Number         |                            | 88    | 105   | 107   | 106   |       |
|              | Pressure, psig     |                            | 948   | 3888  | 3768  | 4400  |       |
|              | Sample Temp., °F.  |                            | 438   | 658   | 701   | 744   |       |
|              | Block Temp., °F.   |                            | 998   | 989   | 993   | 1023  |       |
|              | Sample Wt., gm     |                            | 10.02 | 10.16 | 10.13 | 10.17 |       |
| 12           | Mean Size, $\mu$ m |                            | 31.4  | 20.7  | 21.6  | 17.1  |       |
|              | Run Number         |                            | 89    | 90    | 108   | 110   | 111   |
|              | Pressure, psig     |                            | 680   | 728   | 2784  | 5200  | 5520  |
|              | Sample Temp., °F.  |                            | 354   | 314   | 458   | 799   | 799   |
|              | Block Temp., °F.   |                            | 1004  | 1004  | 998   | 1013  | 1004  |
|              | Sample Wt., gm     |                            | 12.04 | 12.01 | 12.02 | 12.08 | 11.95 |
|              | Mean Size, $\mu$ m |                            | 21.2  | 34.1  | 23.9  | 24.7  | 7.09  |
|              | Run Number         |                            | 92    | 91    | 112   | 113   | 114   |
| 14           | Pressure, psig     |                            | 1320  | 2400  | 5632  | 6576  | 5432  |
|              | Sample Temp., °F.  |                            | 221   | 458   | 611   | 756   | 744   |
|              | Block Temp., °F.   |                            | 1002  | 1006  | 975   | 996   | 981   |
|              | Sample Wt., gm     |                            | 14.01 | 14.03 | 14.30 | 14.15 | 14.19 |
|              | Mean Size, $\mu$ m |                            | 34.2  | 27.6  | 26.3  | 23.3  | 21.7  |
|              | Run Number         |                            | 115   | 116   | 117   | 118   | 119   |
|              | Pressure, psig     |                            | 3280  | 4576  | 5904  | 7216  | 7460  |
|              | Sample Temp., °F.  |                            | 296   | 475   | 763   | 756   | 756   |
| 16           | Block Temp., °F.   |                            | 1006  | 1002  | 1002  | 996   | 998   |
|              | Sample Wt., gm     |                            | 16.04 | 16.13 | 15.99 | 16.02 | 16.21 |
|              | Mean Size, $\mu$ m |                            | 29.4  | 26.2  | 25.0  | 21.0  | 22.1  |

TABLE XIV

|              |                    | 1200° F. Block Temperature |      |       |      |       |       |       |
|--------------|--------------------|----------------------------|------|-------|------|-------|-------|-------|
| Wt. set, gms | Value              | Time Set, Minutes          |      |       |      |       |       |       |
|              |                    | 1                          | 2    | 3     | 5    | 7     |       |       |
| 4            | Run Number         | 74                         | 76   | 75    | 81   | 120   | 121   | 122   |
|              | Pressure, psig     | 640                        | 512  | 1392  | 1428 | 2216  | 2384  | 2256  |
|              | Sample Temp., °F.  | 455                        | 431  | 699   | 714  | 867   | 869   | 842   |
|              | Block Temp., °F.   | 1171                       | 1206 | 1207  | 1186 | 1192  | 1165  | 1142  |
|              | Sample Wt., gm     | 4.01                       | 4.02 | 4.04  | 4.01 | 3.95  | 3.97  | 4.01  |
|              | Mean Size, $\mu$ m | 19.8                       | 28.5 | 22.4  | 28.0 | 19.6  | 17.8  | 21.0  |
|              | Run Number         | 77                         |      | 82    |      | 123   | 124   | 125   |
|              | Pressure, psig     | 720                        |      | 1656  |      | 3760  | 3824  | 3680  |
| 6            | Sample Temp., °F.  | 417                        |      | 557   |      | 913   | 884   | 850   |
|              | Block Temp., °F.   | 1214                       |      | 1190  |      | 1205  | 1172  | 1165  |
|              | Sample Wt., gm     | 6.03                       |      | 6.01  |      | 5.96  | 5.91  | 5.96  |
|              | Mean Size, $\mu$ m | 28.8                       |      | 27.9  |      | 17.2  | 13.8  | 7.69  |
|              | Run Number         | 78                         |      | 83    |      | 126   | 127   | 129   |
|              | Pressure, psig     | 620                        |      | 2640  |      | 4696  | 5856  | 5088  |
|              | Sample Temp., °F.  | 393                        |      | 576   |      | 892   | 899   | 850   |
|              | Block Temp., °F.   | 1197                       |      | 1193  |      | 1165  | 1173  | 1104  |
| 8            | Sample Wt., gm     | 8.01                       |      | 8.03  |      | 8.21  | 8.08  | 8.07  |
|              | Mean Size, $\mu$ m | 24.6                       |      | 20.3  |      | 16.3  | 15.8  | 15.4  |
|              | Run Number         | 128                        |      | 84    |      | 130   | 131   | 132   |
|              | Pressure, psig     | 1144                       |      | 5360  |      | 5776  | 5856  | 7240  |
|              | Sample Temp., °F.  | 296                        |      | 669   |      | 884   | 842   | 943   |
|              | Block Temp., °F.   | 1158                       |      | 1207  |      | 1212  | 1159  | 1199  |
|              | Sample Wt., gm     | 10.14                      |      | 10.01 |      | 10.00 | 10.00 | 9.99  |
|              | Mean Size, $\mu$ m | 30.6                       |      | 17.6  |      | 15.5  | 15.7  | 17.6  |
| 10           | Run Number         | 79                         |      | 133   |      | 134   | 135   | 161   |
|              | Pressure, psig     | 1288                       |      | 5072  |      | 7008  | 7300  | 7200  |
|              | Sample Temp., °F.  | 379                        |      | 467   |      | 799   | 871   | 870   |
|              | Block Temp., °F.   | 1192                       |      | 1184  |      | 1163  | 1159  | 1235  |
|              | Sample Wt., gm     | 12.03                      |      | 12.09 |      | 12.20 | 12.25 | 12.00 |
|              | Mean Size, $\mu$ m | 33.5                       |      | 23.8  |      | 18.3  | 19.3  | 13.2  |
|              | Run Number         | 80                         |      | 136   |      | 137   |       |       |
|              | Pressure, psig     | 2160                       |      | 7060  |      | 7580  |       |       |
| 12           | Sample Temp., °F.  | 287                        |      | 735   |      | 761   |       |       |
|              | Block Temp., °F.   | 1180                       |      | 1161  |      | 1159  |       |       |
|              | Sample Wt., gm     | 14.01                      |      | 14.18 |      | 14.07 |       |       |
|              | Mean Size, $\mu$ m |                            |      |       |      |       |       |       |
| 14           | Run Number         |                            |      |       |      |       |       |       |
|              | Pressure, psig     |                            |      |       |      |       |       |       |
|              | Sample Temp., °F.  |                            |      |       |      |       |       |       |
|              | Block Temp., °F.   |                            |      |       |      |       |       |       |

TABLE XIV-continued

| Wt. set, gms | Value Identification | 1200° F. Block Temperature |       |       |                                                    |   |
|--------------|----------------------|----------------------------|-------|-------|----------------------------------------------------|---|
|              |                      | 1                          | 2     | 3     | 5                                                  | 7 |
| 16           | Mean Size, $\mu$ m   | 31.4                       | 20.7  | 18.2  |                                                    |   |
|              | Run Number           | 138                        | 159   | 162   | Pressure Would Exceed Equipment Safety Limitations |   |
|              | Pressure, psig       | 4832                       | 7760  | 6800  |                                                    |   |
|              | Sample Temp., °F.    | 332                        | 460   | 615   |                                                    |   |
|              | Block Temp., °F.     | 1201                       | 1250  | 1190  |                                                    |   |
|              | Sample Wt., gm       | 16.21                      | 16.36 | 16.01 |                                                    |   |
|              | Mean Size, $\mu$ m   | 39.0                       | 21.0  | 15.2  |                                                    |   |

TABLE XV

| Wt. Set, gms | Value Identification | 1400° F. Block Temperature |                                                    |      |      |      |
|--------------|----------------------|----------------------------|----------------------------------------------------|------|------|------|
|              |                      | 1                          | 2                                                  | 3    | 5    | 7    |
| 4            | Run Number           | 139                        | 96                                                 | 140  | 141  | 155  |
|              | Pressure, psig       | 2168                       | 3136                                               | 3264 | 3584 | 3904 |
|              | Sample Temp., °F.    | 578                        | 1019                                               | 977  | 998  | 1010 |
|              | Block Temp., °F.     | 1358                       | 1379                                               | 1312 | 1330 | 1329 |
|              | Sample Wt., gm       | 4.50                       | 4.07                                               | 4.07 | 4.12 | 3.98 |
|              | Mean Size, $\mu$ m   | 20.1                       | 11.8                                               | 15.1 | 13.0 | 15.5 |
| 6            | Run Number           | 142                        | 148                                                | 97   | 152  | 153  |
|              | Pressure, psig       | 3080                       | 4680                                               | 2096 | 4528 | 5740 |
|              | Sample Temp., °F.    | 684                        | 970                                                | 820  | 1044 | 1040 |
|              | Block Temp., °F.     | 1308                       | 1336                                               | 1317 | 1410 | 1358 |
|              | Sample Wt., gm       | 6.13                       | 6.02                                               | 6.32 | 6.11 | 6.02 |
|              | Mean Size, $\mu$ m   | 24.7                       | 16.1                                               | 24.3 | 12.1 | 13.4 |
| 8            | Run Number           | 143                        | 149                                                | 156  | 157  |      |
|              | Pressure, psig       | 2744                       | 6096                                               | 4960 | 5440 |      |
|              | Sample Temp., °F.    | 526                        | 865                                                | 994  | 1045 |      |
|              | Block Temp., °F.     | 1330                       | 1373                                               | 1375 | 1358 |      |
|              | Sample Wt., gm       | 8.04                       | 8.20                                               | 8.19 | 8.27 |      |
|              | Mean Size, $\mu$ m   | 26.1                       | 15.2                                               | 7.24 | 13.0 |      |
| 10           | Run Number           | 144                        | 150                                                |      |      |      |
|              | Pressure, psig       | 2448                       | 6904                                               |      |      |      |
|              | Sample Temp., °F.    | 408                        | 825                                                |      |      |      |
|              | Block Temp., °F.     | 1394                       | 1351                                               |      |      |      |
|              | Sample Wt., gm       | 10.19                      | 10.08                                              |      |      |      |
|              | Mean Size, $\mu$ m   | 29.6                       | 16.3                                               |      |      |      |
| 12           | Run Number           | 145                        | 151                                                |      |      |      |
|              | Pressure, psig       | 1360                       | 6768                                               |      |      |      |
|              | Sample Temp., °F.    | 287                        | 690                                                |      |      |      |
|              | Block Temp., °F.     | 1345                       | 1330                                               |      |      |      |
|              | Sample Wt., gm       | 12.07                      | 12.01                                              |      |      |      |
|              | Mean Size, $\mu$ m   | 34.6                       | 19.0                                               |      |      |      |
| 14           | Run Number           | 146                        | 158                                                |      |      |      |
|              | Pressure, psig       | 3440                       | 7680                                               |      |      |      |
|              | Sample Temp., °F.    | 230                        | 965                                                |      |      |      |
|              | Block Temp., °F.     | 1330                       | 1375                                               |      |      |      |
|              | Sample Wt., gm       | 14.11                      | 14.05                                              |      |      |      |
|              | Mean Size, $\mu$ m   | 30.9                       | 13.0                                               |      |      |      |
| 16           | Run Number           | 147                        | Pressure Would Exceed Equipment Safety Limitations |      |      |      |
|              | Pressure, psig       | 7240                       |                                                    |      |      |      |
|              | Sample Temp., °F.    | 442                        |                                                    |      |      |      |
|              | Block Temp., °F.     | 1351                       |                                                    |      |      |      |
|              | Sample Wt., gm       | 16.04                      |                                                    |      |      |      |
|              | Mean Size, $\mu$ m   | 19.4                       |                                                    |      |      |      |

The temperature, pressure and particle size data presented in Tables XIII to XV was segregated and retabulated below in accordance with the specific thermodynamic regimes (superpressured water, superheated steam or supercritical) applicable to a particular data point. The data for the superpressured water appears in Table XVI, the data for superheated steam appears in Table XVII and the data for supercritical conditions appears in Table XVIII.

TABLE XVI

| MEASURED VALUES: SUPERPRESSURED WATER REGION VS. VOLUMETRIC MEAN PARTICLE SIZE |               |                 |               |                   |
|--------------------------------------------------------------------------------|---------------|-----------------|---------------|-------------------|
| Run Number                                                                     | Pressure psig | Temperature, F. | Time, Minutes | Size, Micrometers |
| 74                                                                             | 640           | 455             | 1.0           | 19.8              |

TABLE XVI-continued

| MEASURED VALUES: SUPERPRESSURED WATER REGION VS. VOLUMETRIC MEAN PARTICLE SIZE |               |                 |               |                   |
|--------------------------------------------------------------------------------|---------------|-----------------|---------------|-------------------|
| Run Number                                                                     | Pressure psig | Temperature, F. | Time, Minutes | Size, Micrometers |
| 60                                                                             | 76            | 512             | 431           | 28.5              |
|                                                                                | 77            | 720             | 417           | 28.8              |
|                                                                                | 78            | 620             | 393           | 34.6              |
|                                                                                | 79            | 1288            | 379           | 33.5              |
|                                                                                | 80            | 2160            | 287           | 31.4              |
|                                                                                | 82            | 1656            | 557           | 27.9              |
|                                                                                | 83            | 2640            | 576           | 20.3              |
|                                                                                | 84            | 5360            | 669           | 17.6              |
|                                                                                | 86            | 800             | 431           | 31.4              |
|                                                                                | 87            | 568             | 386           | 35.8              |
|                                                                                | 88            | 948             | 438           | 31.4              |
|                                                                                | 89            | 680             | 354           | 21.2              |

TABLE XVI-continued

| MEASURED VALUES: SUPERPRESSURED WATER REGION VS. VOLUMETRIC MEAN PARTICLE SIZE |                |                  |               |                   |
|--------------------------------------------------------------------------------|----------------|------------------|---------------|-------------------|
| Run Number                                                                     | Pressure, psig | Temperature, °F. | Time, Minutes | Size, Micrometers |
| 90                                                                             | 728            | 314              | 2.0           | 34.1              |
| 91                                                                             | 2400           | 458              | 2.0           | 27.6              |
| 92                                                                             | 1320           | 221              | 1.0           | 34.2              |
| 94                                                                             | 1392           | 572              | 3.0           | 27.1              |
| 95                                                                             | 1560           | 520              | 3.0           | 30.1              |
| 99                                                                             | 412            | 345              | 1.0           | 19.8              |
| 105                                                                            | 3888           | 658              | 3.0           | 20.7              |
| 107                                                                            | 3768           | 701              | 5.0           | 21.6              |
| 108                                                                            | 2784           | 458              | 3.0           | 23.9              |
| 112                                                                            | 5632           | 611              | 3.0           | 26.3              |
| 115                                                                            | 3280           | 296              | 1.0           | 29.4              |
| 116                                                                            | 4576           | 475              | 2.0           | 26.1              |
| 128                                                                            | 1144           | 298              | 1.0           | 30.6              |
| 133                                                                            | 5074           | 467              | 2.0           | 23.8              |
| 138                                                                            | 4832           | 332              | 1.0           | 39.0              |
| 139                                                                            | 2168           | 578              | 1.0           | 20.1              |
| 142                                                                            | 3080           | 684              | 1.0           | 24.7              |
| 143                                                                            | 2744           | 526              | 1.0           | 26.1              |
| 144                                                                            | 2448           | 402              | 1.0           | 29.6              |
| 145                                                                            | 1360           | 287              | 1.0           | 34.6              |
| 146                                                                            | 3440           | 230              | 1.0           | 30.9              |
| 147                                                                            | 7240           | 442              | 1.0           | 19.4              |
| 151                                                                            | 6768           | 690              | 2.0           | 19.0              |
| 159                                                                            | 7760           | 460              | 1.0           | 21.0              |
| 160                                                                            | 6800           | 615              | 2.0           | 12.7              |
| 162                                                                            | 6800           | 615              | 2.0           | 15.2              |
| Mean                                                                           | 2871.5         | 462.4            | 1.69          | 26.41             |
| Std. Dev.                                                                      | 2193.6         | 133.9            | 0.89          | 6.28              |

TABLE XVII

| MEASURED VALUES: SUPERHEATED STEAM VS. VOLUMETRIC MEAN PARTICLE SIZE |                |                  |               |                   |
|----------------------------------------------------------------------|----------------|------------------|---------------|-------------------|
| Run Number                                                           | Pressure, psig | Temperature, °F. | Time, Minutes | Size, Micrometers |
| 75                                                                   | 1392           | 699              | 2.0           | 22.4              |
| 81                                                                   | 1428           | 714              | 2.0           | 28.0              |
| 85                                                                   | 504            | 513              | 2.0           | 27.6              |
| 93                                                                   | 1200           | 677              | 3.0           | 27.6              |
| 96                                                                   | 3136           | 1019             | 2.0           | 11.8              |
| 97                                                                   | 2096           | 820              | 3.0           | 24.3              |
| 98                                                                   | 1256           | 628              | 7.0           | 21.0              |
| 100                                                                  | 1952           | 694              | 5.0           | 24.3              |
| 101                                                                  | 2208           | 710              | 7.0           | 22.3              |
| 102                                                                  | 2284           | 750              | 5.0           | 23.4              |
| 103                                                                  | 3176           | 708              | 7.0           | 22.3              |
| 104                                                                  | 3000           | 705              | 5.0           | 23.0              |
| 109                                                                  | 1332           | 662              | 5.0           | 24.1              |
| 120                                                                  | 2216           | 867              | 3.0           | 19.6              |
| 121                                                                  | 2384           | 869              | 5.0           | 17.8              |
| 122                                                                  | 2256           | 842              | 5.0           | 21.0              |
| Mean                                                                 | 1988.7         | 742.3            | 4.37          | 22.53             |
| Std. Dev.                                                            | 759.0          | 118.1            | 1.96          | 4.02              |

TABLE XVIII

| MEASURED VALUES: SUPERCRITICAL WATER REGION VS. VOLUMETRIC MEAN PARTICLE SIZE |                |                  |               |                   |
|-------------------------------------------------------------------------------|----------------|------------------|---------------|-------------------|
| Run Number                                                                    | Pressure, psig | Temperature, °F. | Time, Minutes | Size, Micrometers |
| 106                                                                           | 4400           | 744              | 7.0           | 17.1              |
| 110                                                                           | 5200           | 799              | 5.0           | 24.7              |
| 111                                                                           | 5520           | 799              | 7.0           | 7.09              |
| 113                                                                           | 6576           | 756              | 5.0           | 23.3              |
| 114                                                                           | 6432           | 744              | 7.0           | 21.7              |
| 117                                                                           | 5904           | 763              | 3.0           | 25.0              |
| 118                                                                           | 7216           | 756              | 5.0           | 21.0              |
| 119                                                                           | 7460           | 756              | 7.0           | 22.0              |
| 123                                                                           | 3760           | 913              | 3.0           | 17.2              |
| 124                                                                           | 3824           | 884              | 5.0           | 13.8              |
| 125                                                                           | 3680           | 850              | 7.0           | 7.69              |
| 126                                                                           | 4696           | 802              | 3.0           | 16.3              |
| 127                                                                           | 5856           | 899              | 5.0           | 15.8              |
| 129                                                                           | 5088           | 850              | 7.0           | 15.4              |

TABLE XVIII-continued

| MEASURED VALUES: SUPERCRITICAL WATER REGION VS. VOLUMETRIC MEAN PARTICLE SIZE |                |                  |               |                   |
|-------------------------------------------------------------------------------|----------------|------------------|---------------|-------------------|
| Run Number                                                                    | Pressure, psig | Temperature, °F. | Time, Minutes | Size, Micrometers |
| 130                                                                           | 5776           | 884              | 3.4           | 15.5              |
| 131                                                                           | 5856           | 842              | 3.0           | 15.7              |
| 132                                                                           | 7064           | 943              | 5.0           | 17.6              |
| 134                                                                           | 7008           | 799              | 3.0           | 18.3              |
| 135                                                                           | 7300           | 871              | 3.9           | 19.3              |
| 136                                                                           | 7060           | 735              | 2.0           | 20.7              |
| 137                                                                           | 7580           | 761              | 3.0           | 18.2              |
| 140                                                                           | 3264           | 977              | 3.0           | 15.1              |
| 141                                                                           | 3584           | 998              | 5.0           | 13.0              |
| 148                                                                           | 4680           | 970              | 2.0           | 16.1              |
| 149                                                                           | 6096           | 865              | 2.0           | 15.2              |
| 150                                                                           | 6904           | 825              | 2.0           | 16.3              |
| 152                                                                           | 4528           | 1044             | 5.0           | 12.1              |
| 153                                                                           | 5740           | 1044             | 5.0           | 13.4              |
| 156                                                                           | 4960           | 994              | 3.0           | 7.24              |
| 157                                                                           | 5440           | 1045             | 5.0           | 13.0              |
| 158                                                                           | 7680           | 965              | 2.0           | 13.0              |
| 161                                                                           | 7200           | 870              | 5.0           | 13.2              |
| Mean                                                                          | 5729.1         | 869.8            | 4.32          | 16.28             |
| Std. Dev.                                                                     | 1322.5         | 97.0             | 1.70          | 4.54              |

25 The data tabulated in Tables XVI, XVII and XVIII was subjected to computer analysis by a least squares regression analysis program to determine if the measured dependent variable of mean particle size could be correlated in any manner to the measured values of time, pressure and temperature. The independent variables specifically selected in an attempt to develop a correlation having greater than a 90% confidence level are Pressure, P; Temperature, T; Time,  $\theta$ ; Pressure times temperature; Pressure times time; Temperature times time; Pressure squared; Temperature squared; Time squared; Natural logarithm of pressure; Natural logarithm of temperature and Natural logarithm of time.

30 The correlation obtained for the superpressured water regime (Table XVI) is:

35 The correlation obtained for the superheated steam regime (Table XVII) is:

Volumetric Mean Particle Size, micrometers =

$$45 \quad 38.35929 + 2.9416 \left( \ln \frac{P}{1000} \right) - 5.51285 \left( \ln \frac{T}{100} \right) - 0.40358 \left( \frac{P \times T}{100,000} \right)$$

50 where P=pressure, psig and T=temperature, °F.

The correlation coefficient is  $r=0.7539$  with a standard estimate of error  $s_c=4.2992$  micrometers.

55 The analysis of variance table is:

|               | Degrees of Freedom | Sum of Squares | Mean Square | F Ratio |
|---------------|--------------------|----------------|-------------|---------|
| 60 Regression | 2                  | 801.939        | 400.970     | 20.724  |
| Residual      | 36                 | 696.540        | 19.348      |         |

An F ratio greater than 4 indicates that the correlation is statistically significant and reliable. The specific F ratio obtained provides a confidence level greater than 0.999.

65 The correlation obtained for the superheated steam regime (Table XVII) is:

Volumetric Mean Particle Size, micrometers =  $2.12238 +$ 

$$9.81236 \left( \frac{T}{100} \right) - 0.82034 \left( \frac{T}{100} \right)^2 - 0.08391 (\theta)^2 \quad 5$$

where  $T$ =temperature, °F. and  $\theta$ =time, minutesThe correlation coefficient is  $r=0.9071$  with a standard estimate of error  $s_e=2.2254 \mu\text{m}$ . 10

The analysis of variance table is:

|            | Degrees of Freedom | Sum of Squares | Mean Square | F Ratio | 15 |
|------------|--------------------|----------------|-------------|---------|----|
| Regression | 3                  | 199.078        | 66.359      | 18.581  |    |
| Residual   | 12                 | 42.857         | 3.571       |         |    |

The F ratio obtained provided a confidence level greater than 0.999.

The correlation obtained for the supercritical fluid regime (Table XVIII) is: 20

Volumetric Mean Particle Size, micrometers =

$$267.50971 + 18.60361 \left( \frac{T}{100} \right) +$$

$$4.86879 (\theta) - 0.61985 (\theta)^2 - 195.05659 \left( \ln \frac{T}{100} \right) \quad 30$$

where  $T$ =temperature, °F. and  $\theta$ =time, minutes.The correlation coefficient is  $r=0.7498$  with a standard estimate of error  $s_e=3.2176 \mu\text{m}$ . 35

The analysis of variance table is:

|            | Degrees of Freedom | Sum of Squares | Mean Square | F Ratio | 40 |
|------------|--------------------|----------------|-------------|---------|----|
| Regression | 4                  | 358.931        | 89.733      | 8.667   |    |
| Residual   | 27                 | 279.528        | 10.353      |         |    |

This F ratio obtained provides a confidence level greater than 0.999. 45The actual results obtained in the supercritical regime are compared, in Table XIX, to the results that would be predicted from each of these separate correlations developed for the three separate thermodynamic regimes. In addition, each of these correlations are plotted, in graphical form in FIGS. 12 and 13. 50

TABLE XIX

| SUPERCritical REGIME MEASURED DATA COMPARED WITH PREDICTION CALCULATED VALUES FROM CORRELATIONS |                                 |                              |               |             |
|-------------------------------------------------------------------------------------------------|---------------------------------|------------------------------|---------------|-------------|
| Run Number                                                                                      | Measured Mean Size, Micrometers | Calculated Size, Micrometers |               |             |
|                                                                                                 |                                 | Supercritical                | Super-pressed | Superheated |

|     |      |      |      |      |    |
|-----|------|------|------|------|----|
| 106 | 17.1 | 18.2 | 18.4 | 21.4 | 60 |
| 110 | 24.7 | 19.6 | 15.0 | 21.8 |    |
| 111 | 7.09 | 14.5 | 14.1 | 19.8 |    |
| 113 | 23.3 | 22.4 | 12.7 | 23.1 |    |
| 114 | 21.7 | 18.2 | 13.5 | 21.4 |    |
| 117 | 25.0 | 22.1 | 14.2 | 24.2 |    |
| 118 | 21.0 | 22.4 | 11.0 | 23.1 | 65 |
| 119 | 22.0 | 17.3 | 10.4 | 21.1 |    |
| 123 | 17.2 | 15.0 | 16.2 | 18.3 |    |
| 124 | 13.8 | 15.7 | 16.6 | 18.4 |    |
| 125 | 7.69 | 11.9 | 17.8 | 17.9 |    |

TABLE XIX-continued

## SUPERCritical REGIME MEASURED DATA COMPARED WITH PREDICTION CALCULATED VALUES FROM CORRELATIONS

| Run Number                                          | Measured Mean Size, Micrometers | Calculated Size, Micrometers |               |               |
|-----------------------------------------------------|---------------------------------|------------------------------|---------------|---------------|
|                                                     |                                 | Micro-meters                 | Supercritical | Super-pressed |
| 126                                                 | 16.3                            | 15.6                         | 13.9          | 19.4          |
| 127                                                 | 15.8                            | 15.2                         | 10.2          | 17.7          |
| 129                                                 | 15.4                            | 11.9                         | 13.9          | 17.9          |
| 130                                                 | 15.5                            | 16.3                         | 10.9          | 19.5          |
| 131                                                 | 15.7                            | 17.6                         | 11.9          | 21.6          |
| 132                                                 | 17.6                            | 14.1                         | 4.9           | 15.4          |
| 134                                                 | 18.3                            | 19.8                         | 10.0          | 23.2          |
| 135                                                 | 19.3                            | 16.9                         | 6.6           | 19.8          |
| 136                                                 | 20.7                            | 22.4                         | 12.2          | 25.3          |
| 137                                                 | 18.2                            | 22.3                         | 9.8           | 24.3          |
| 140                                                 | 15.1                            | 13.7                         | 16.4          | 14.7          |
| 141                                                 | 13.0                            | 13.3                         | 15.0          | 12.0          |
| 148                                                 | 16.1                            | 12.0                         | 12.1          | 15.5          |
| 149                                                 | 15.2                            | 14.8                         | 10.5          | 21.0          |
| 150                                                 | 16.3                            | 16.6                         | 9.4           | 22.7          |
| 152                                                 | 12.1                            | 13.0                         | 10.8          | 8.8           |
| 153                                                 | 13.4                            | 13.1                         | 6.4           | 8.8           |
| 156                                                 | 7.24                            | 13.5                         | 10.5          | 13.6          |
| 157                                                 | 13.0                            | 13.0                         | 7.5           | 8.7           |
| 158                                                 | 13.0                            | 12.1                         | 1.9           | 15.8          |
| 161                                                 | 13.2                            | 16.2                         | 7.0           | 19.1          |
| Mean                                                | 16.28                           | 16.27                        | 11.62         | 18.60         |
| Std. Dev.                                           | 4.54                            | 3.40                         | 3.82          | 4.55          |
| Student's "t" Value                                 |                                 | -0.012                       | 2.893         | -5.816        |
| Probability that data is from different populations |                                 | <0.51                        | <0.995        | <0.9995       |

As evidenced by the comparisons contained in Table XIX and the graphical representations set forth in FIGS. 12 and 13, it is not possible to accurately predict the results obtained in the supercritical regime from data obtained in the superheated steam and superpressured water regimes. For example, based on the student "t" values set forth, the probability is less than 5 chances in 1000 that the results obtained in the superheated steam and superpressured water regimes can accurately predict the results to be expected in the supercritical regimes.

In addition to evaluating the effect of pressure and temperature on particle size in accordance with the test procedure just described, the effect of the addition of an electrolyte on particle size was investigated. The results obtained are set forth in Table XX below:

TABLE XX

## EFFECT OF ELECTROLYTE ON VOLUMETRIC MEAN PARTICLE SIZE REDUCTION

| Run Number               | Pres-<br>sure,<br>psig | Temper-<br>ature,<br>°F. | Time,<br>Minutes | g/liter and<br>Electrolyte | Mean Size,<br>Micrometers |
|--------------------------|------------------------|--------------------------|------------------|----------------------------|---------------------------|
|                          |                        |                          |                  |                            | 55                        |
| Basic feed material size |                        |                          |                  |                            | 50.6                      |
| 134                      | 7008                   | 799                      | 3.0              | None                       | 18.3                      |
| 135                      | 7300                   | 871                      | 3.9              | None                       | 19.3                      |
| 165                      | 7000                   | 800                      | 2.6              | 0.37 NaCl                  | 14.6                      |
| 166                      | 6800                   | 695                      | 3.0              | 0.37 NaCl                  | 13.5                      |
| 167                      | 6250                   | 800                      | 3.0              | 0.13 NaOH                  | 5.15                      |
| 168                      | 5700                   | 800                      | 3.0              | 0.13 NaOH                  | 5.23                      |
| 169                      | 6400                   | 800                      | 3.0              | 1.2 NaOH                   | 11.4                      |
| 170                      | 8650                   | 805                      | 3.0              | 1.2 NaOH                   | 7.01                      |
| 171                      | 7700                   | 750                      | 3.0              | 1.2 NaOH                   | 11.5                      |

The data contained in Table XX shows that the addition of electrolyte appreciably increases the degree of comminution obtained, i.e. smaller particle sizes are obtained.

DETAILED DESCRIPTION OF  
PARTICULARLY PREFERRED EMBODIMENT

FIG. 5 illustrates a particularly preferred embodiment of the process for the present invention for large scale coal comminution and mineral removal. In this process, the overall system 10 includes a pair of slurry holding tanks 22, 23 for mixing the pulverized coal with water by mechanical stirrers 24, 25. Two tanks 22, 23 are preferred so that the system 10 will have an alternate supply as one tank empties. As indicated previously, the system 10 may use any porous or fluid-permeable, friable solid, especially coal, and any liquid which is compatible both with the formation of a slurry and with the components of the process and system 10.

It is noted that coal slurries of greater than about 18 percent solids content from non-Newtonian fluids which are highly viscous and may be difficult to pump. The minimum amount of water which may be used in the invention equals the amount necessary to fill the pores of the coal and the interstitial spaces between the coal particles. Particularly preferred are slurries of coal and water and/or a low molecular weight alcohol such as methanol. The slurry composition preferably has a pumpable solids content that varies with coal particle size distribution, but generally of less than about 55 percent, preferably between about 40 and about 55 percent dry coal at ordinary ambient temperature.

Two slurry lines 26, 27 lead from the tanks 22, 23 to a three way valve 28 where the two lines 26, 27 are merged and fed into a circulating pump 30. Circulating pump 30 draws a slurry from either tank 22 or 23 and delivers it via line 32 to the feed pump 34. Line 32 is also connected to an additional slurry line 36 which leads to a second three way valve 38. The second valve 38 separates and directs the flow of line 36 to either tank 22 or 23 via lines 40 or 41.

Lines 26, 27, 32, 36, 40 and 41 form a loop around the tanks 22, 23. Circulating pump 30 operates continuously pumping a flow of slurry through a loop with the advantage that the continuous stirring action of mixers 24, 25 and pump 30 provide a uniform and consistent composition of the feed. The slurry is drawn off this loop through line 32 by feed pump 34 for delivery to the reactor at a high, constant pressure.

As previously mentioned, it is advantageous to add a predetermined amount of electrolyte solution to the slurry in order to control the electrical resistance of the slurry. In preferred form, FIG. 5 shows a proportioning pump 42 feeding a predetermined amount of electrolyte solution into the slurry through a line 44. The electrolyte is preferably a hydroxide, such as sodium hydroxide, calcium hydroxide or ammonium hydroxide, but may be any electrolyte desired. It is desirable to add the electrolyte solution prior to the feed pump 34 so that proportioning pump 42 does not have to operate in opposition to high operating pressures.

Referring again to FIG. 5, a constant pressure pumping system, generally 14, of the present invention provides a system for delivering slurry to the process at constant pressure. The constant pressure pumping system 14 counteracts sudden or severe pressure changes within the system 10 by increasing the rate of slurry fed to the system 10 as the pressure within the system 10 decreases or, alternatively, decreasing the rate at which slurry is fed to the system 10 as the pressure increases.

The constant pressure pumping system 14 includes a pump 46 preferably driven by a constant speed motor 50

through a drive connection 52 to deliver hydraulic fluid from a reservoir 48 to a hydraulic motor 54. The resultant hydraulic fluid flow is passed through a hydraulic motor 54 which is used to drive feed pump 34 thereby producing a pressure drop across the hydraulic motor. The hydraulic motor 54 produces a driving force which is directly proportional to the amount of pressure drop which is produced across the motor 54.

A pressure sensitive flow control valve 56 is used to control the flow of hydraulic fluid to the hydraulic motor 54. As the pressure drop across the hydraulic motor 54 increases, the pressure sensitive valve 56 decreases the flow of hydraulic fluid through the hydraulic motor 54 in order to decrease the pressure drop across the hydraulic motor 54 to a predetermined level. As the pressure drop across the hydraulic motor 54 decreases, the flow from the hydraulic pump 46 through the hydraulic motor 54 increases. In the preferred embodiment, the flow control valve 56 controls the angle of a swash plate contained within the pump 46 thereby increasing or decreasing the volume of fluid pumped by pump 46 as needed.

The valve varies the amount of hydraulic fluid flowing to the hydraulic motor 54 thereby maintaining a substantially constant pressure drop across the hydraulic motor 54. As a result, a substantially constant driving force is generated by the hydraulic motor 54.

The hydraulic motor 54 acts through a second drive connection 58 to drive the feed pump 34 which has a delivery pressure directly proportional to the amount of driving force generated by the hydraulic motor 54. Since this driving force is maintained constant, the delivery pressure of the fluid, such as a coal-water slurry is also maintained constant; the flow rate of the fluid is reduced as pressure within the system 10 is increased and vice versa. The constant pressure pumping system 14 thereby acts to counteract pressure changes within the system 10, to prevent explosion or damage to the constant pressure pumping system 14 and to protect the integrity of the feed pump 34.

The hydraulic fluid pump 46, the hydraulic motor 54 and the pressure sensing flow control valve 56 form an indirect control of the constant pressure pumping system 14. This constant pressure pumping system 14 is preferred for use in delivering abrasive slurries such as slurries of coal and water because the abrasive feed slurry never contacts the pressure sensing valve 56, thus greatly extending the useful life of the control loop and valve 56.

The feed pump 34 is preferably a positive displacement type of pump, such as a piston or plunger design pump. Pumps of this design are well suited to delivering the high operating pressures necessary for explosive comminution. Because of the highly abrasive nature of coal slurries, it was necessary to provide a specifically designed pump cylinder and valve assembly of the feed pump 34.

In order to prevent a dangerous and damaging pressure build up exceeding the design strength of the process, a pressure relief system 74 is attached to slurry line 72 which delivers slurry from the feed pump 34 to the rest of the system 10. It has been found that an abrupt drop in the high pressure in the system 10 or a stoppage of slurry flow through the system causes rapid agglomeration of the hot slurry solids and setting of the particulate coal solids into a solid fused mass within the system 10. The pressure relief system 74 is designed to mini-

mize solids agglomeration and flow stoppage of the coal slurry within the system 10.

The pressurized slurry in line 72 is delivered to the heating unit 79 which preferably includes three sequential heating chambers 80, 81 and 82 connected by lines 84 and 85. The temperature of the slurry is preferably measured, for example, by thermocouples 86, 87, 88 and 98 and pressure by gauges 91, 92 and 95 and electrical conductivity by meter 90. The information provided about conditions within the heating units 80, 81 and 82 enables an operator of the system 10 to determine, for example, whether to increase or decrease the amount of energy passed through the slurry by varying the amount of electrolyte mixed into the slurry by proportioning pump 42.

The preferred form for the heating unit 79 is shown in FIG. 6. The heating unit 79 comprises electrically conducting cylindrical containers 150, 151 and 152 grounded in an conventional manner by wire 153 to act as an electrode. Each container has an inlet 154, 155 and 156 and an outlet 158, 159 and 160, respectively. Cylindrical electrodes 162, 163 and 164 are mounted within the interior of each cylinder 150, 151 and 152, respectively. The length of the electrodes 162, 163 and 164 is nearly equal to the internal length of the cylinders 150, 151 and 152. The electrodes 162, 163 and 164 are connected preferably to separate phases of a three phase electrical source 165 operating at between about 100 to about 1200 amperes and about 208 to about 480 volts, alternating current when coal is processed at a rate of from 2 to 10 tons/day in unit 79.

Current is passed between electrodes 162, 163 and 164 and the cylinders 150, 151 and 152 as the slurry is passed through the cylinders, thus using the electrical resistance of the slurry as the heating element of the heating units 79. The rate of heating of the slurry is directly proportional to the rate of dissipation of electrical power within the slurry. This system has demonstrated a heating capacity of 5.4 million BTU/hr. ft<sup>3</sup> of available heating unit volume or over 1,000,000 BTU/hr ft<sup>2</sup> of conductor surface. The rate of dissipation of electrical power is related to the resistance of the slurry ( $P=EI=RI^2$ ) so that, as previously explained, the rate of heating of the slurry, assuming constant voltage E, can be simply and effectively controlled by increasing or decreasing R by means of the amount of electrolyte added via proportioning pump 42.

At relatively high operating temperatures and at high solids concentration coating of the electrodes 162, 163 and 164 by material in the slurry becomes a problem. This coating has a high resistivity which fouls the electrodes 162, 163 and 164 and reduces the flow of electrical current. As a result, the temperature of the slurry drops continuously and loss of process control follows. The severity of this problem varies with the type of coal and the solids content of the slurry. Analysis of this coating indicates it is principally a coal substance of somewhat enhanced ash content. The preferred way of minimizing the coating is to operate at a lower solids content and/or higher temperatures and pressures.

It was necessary to provide a specially designed device to pass large electrical currents to the electrodes 162, 163 and 164 within the heating unit 79 of FIG. 5 at the preferred high temperature and high pressure operating conditions.

The pressurized heated slurry is passed from the heating unit 79 (FIG. 5) through slurry line 93 to the expansion unit 94. As stated previously, at preferred operating

temperatures, the necessary residence time is provided by passage of the slurry within the heating chambers 80, 81 and 82, however, slurry line 93 can provide additional residence time, if necessary. Operating conditions at the expansion unit 94 are measured by thermocouple 98 and pressure gauge 95.

Conventional expansion orifices are deficient for use in connection with this invention because they fail to minimize adequately the length of time for the pressure drop to occur (for maximum violence of the explosion and shattering of particles). Specifically, the prior art design is such that the explosive force is partially lost because of a more gradual release of the fluid pressure from within the pores of the coal. In addition, conventional expansion orifices are not designed to withstand the abrasiveness of high temperature, high pressure coal slurries and, as a result, they wear or abrade to become unsuitable for use in a relatively short time. Furthermore, the mixture which is passed from a system for accomplishing explosive comminution at supercritical conditions emerges from the opening of the orifice in an exploding hemispherical pattern, expanding in all directions up to 135° from the direction of flow through the opening. Conventional expansion orifices generally fail in respect to the latter characteristic because they are of a converging/diverging design, similar to a venturi, which design limits the rate of expansion of the slurry and reduces the force of the selective comminution action of the process in the manner previously explained. The adiabatic expansion orifice designed for use with this invention provides for a substantially instantaneous reduction of the pressure in the process. The orifice 94 provides that the slurry will pass across the opening 188 in less than about 10 microseconds, preferably in less than about 1 microsecond and most preferably in less than about 0.3 microsecond. In theory the total amount of time necessary for the pressure drop to occur is equal to the length of time necessary to traverse the orifice length plus the length of time for pressure imposed on the material to equilibrate outside the orifice 94 to downstream pressure conditions. For the orifice design of this invention, that total time is less than about 100 microseconds, preferably less than about 10 microseconds and most preferably less than about 1 microsecond.

A duct 102 is fitted around the orifice 94 to collect the shattered product 100. Duct 102 is preferably designed to provide a minimum distance from the orifice opening 188 which is greater than twenty times the diameter of opening 188. This spacing will avoid interference with the selectivity of the comminution operation of the system 10. The duct 102 may be connected to deliver the product 100 to various subsequent recovery or treatment systems.

The product 100 exiting from the orifice 94 is no longer in slurry form but rather is preferably a water vapor suspension of small hydrocarbonaceous and mineral particles. The water in the slurry will convert, at equilibrium, to steam, liquid water or a mixture thereof depending on the energy content of the water prior to expansion and upon the final pressure, which determines the final temperature. Preferably, the water is completely vaporized in the explosion for maximum shattering and to permit fractionation of the hydrocarbon fraction from the mineral fraction without interference from the droplets of condensate. Therefore, the temperature in the duct 102 is preferably maintained above the dew point of the vapor at the particular pres-

sure existing within the duct 102. The preferred temperature at atmospheric pressure is between about 220° F. and about 275° F.

The product mixture can be drawn from the system 10 at this point by line 96 and used directly or it can be sent through various recovery and processing units as will be explained shortly. The stream of material emerging from the orifice 94 can be passed preferably after separation of the mineral material to a combustion zone, i.e. fired, and used directly as a source of heat. Alternatively, the product could be condensed, recovered and sold to manufacturers for processing and use. Other means of recovery of fuel values may be employed.

In the preferred embodiment shown in FIG. 5, the duct 102 leads to a cyclone 104 having a temperature 15 above the dew point of the vapor, preferably about 250° F. so that no condensation occurs. The hydrocarbonaceous particles of the shattered product have sufficiently smaller size and lower density than the mineral particles of the shattered product so that these two 20 fractions can be fractionated by gravity separation techniques such as through the use of a centrifuge. The hydrocarbon, still suspended in water vapor, is drawn off and sent to condensing, drying, combustion or other processing units 106.

In a preferred embodiment, the hydrocarbonaceous particles can be admixed with a liquid fuel, such as gasoline, fuel oil, residual oil, etc., to extend the fuel value of the liquid fuel.

Because of the difference in the density of the hydrocarbon particles versus the mineral particles as produced by this invention, the cyclone 104 can fractionate the mineral particle fraction having a mean particle size of about 3 microns in diameter from the fraction of hydrocarbon particles having a mean particle size of 35 about 5 microns in diameter.

This fractionation can accomplish the removal of at least a portion of the minerals originally present in the raw feed coal. With a suitable solid scavenger for sulfur, about 85 percent of the sulfur originally present may be removed. Specifically, about 90 percent of the inorganic sulfur and about 80 percent of the organic sulfur may be removed. The minerals and solid sulfur scavenging compounds are drawn off the bottom of the cyclone and provide a potential source of several elements, including, iron, silicon, sulfur, vanadium, germanium and uranium. Alumina and quartz are also potentially useful by-products.

The above description relates to a preferred embodiment of the invention. However, alternative configurations and modifications are possible within the scope of the invention. For example, different pumps or pumping systems may be designed to produce the necessary reactor pressure. Methods of heating the slurry to supercritical conditions, other than passing an electric current through the slurry, may be devised. The heating unit 79 may consist of a single chamber, rather than the three chambers 80, 81 and 82 as shown. Different liquid solutions may be used to make the slurry such as methanol. In addition, it may be desirable in some instances to 60 use a liquefied gas in forming the slurry and to heat the slurry by simply allowing the slurry to reach ambient temperature. Solids other than coals, such as coke or coal char may be used in making the slurry. Gasification reactors or other reactors may be adapted to receive the 65 shattered product directly from the orifice 188. Therefore, the subject matter of the invention is to be limited only by the following claims and their equivalents:

We claim:

1. A material comprising the comminuted product of a slurry of coal having mineral and hydrocarbonaceous material contained therein and a slurry liquid initially maintained at a pressure and temperature above the critical temperature and pressure of the slurry liquid wherein the pressure imposed upon the slurry is subsequently reduced substantially instantaneously to a pressure below the critical pressure of the liquid, the comminuted product comprising a hydrocarbonaceous fraction of discrete particles of hydrocarbonaceous material having
  - (a) a volumetric mean particle size of less than about 5 microns in diameter;
  - (b) a solubility in a solvent selected from the group consisting of gasoline, benzene, methyl alcohol, carbon tetrachloride and tetralin of about two times to about six times greater than the solubility of the original coal;
  - (c) a subtraction of discrete hydrocarbonaceous particles substantially free of sulfur having particle size of less than about 2 microns in diameter;
  - (d) a density of about 50% to 75% of the density of the feed coal;
  - (e) an oxidation decomposition rate determined by thermogravimetric analysis in ambient atmosphere which includes a first peak of about 300° C. and a second peak between about 350° and about 450° C., said decomposition rate decreasing to substantially zero between said first peak and said second peak and,
  - (f) a mineral fraction comprising discrete particles of mineral matter substantially scissioned from the hydrocarbonaceous material having a volumetric mean particle size substantially the same as the mineral matter present in the original coal.
2. A material as in claim 1 wherein the slurry liquid is water.
3. A material as in claim 1 wherein the slurry liquid is 40 water and the slurry is at a temperature of about 750° F. to about 950° F. and a pressure of about 4,000-16,000 psia prior to pressure reduction.
4. The material as in claim 1 wherein the hydrocarbonaceous fraction has a density of about 0.7 to about 0.9 g/cc.
5. A hydrocarbonaceous material derived from coal characterized as being relatively free of mineral components originally present in the coal, and having
  - (a) a volumetric mean particle size of less than about 5 microns,
  - (b) a density of about 0.7 to about 0.9 g/cc,
  - (c) a solubility in a solvent selected from the group consisting of gasoline, benzene, methyl alcohol, carbon tetrachloride and tetralin of about two times to about six times greater than the solubility of the original coal,
  - (d) a subtraction of discrete hydrocarbonaceous particles substantially free of sulfur having a particle size of less than about 2 microns in diameter and,
  - (e) an oxidation decomposition rate determined by thermogravimetric analysis in ambient atmosphere which includes a first peak at about 300° C. and a second peak between about 350° and about 450° C., said decomposition rate decreasing to substantially zero between said first peak and said second peak,
  - (f) said carbonaceous material further comprising the hydrocarbonaceous portion of the explosively comminuted product of a slurry of coal and a liquid

initially maintained at a temperature and pressure above the critical temperature and pressure of the liquid and subsequently comminuted by substantially instantaneously reducing the pressure imposed upon the slurry, said hydrocarbonaceous material being substantially scissioned from the mineral matter originally present in the coal.

6. An admixture of the material of claim 5 with a liquid fuel.

7. An admixture of the material of claim 5 with a vapor.
8. An admixture of the material of claim 7 wherein the vapor is steam.
- 5 9. A material as in claim 5 wherein the slurry liquid is water.

10. A material as in claim 5 wherein the slurry liquid is water and the slurry is at a temperature of about 750° F. to about 950° F. and a pressure of about 4,000-16,000 psia prior to pressure reduction.

\* \* \* \* \*

15

20

25

30

35

40

45

50

55

60

65